# EUROPEAN PATENT APPLICATION

(11) **EP 4 741 153 A1**
(43) Date of publication of application: **13.05.2026**
(21) Application number: 24836076.0
(22) Date of filing: 03.07.2024
(51) Int. Cl.: B32B 15/08, B32B 15/18, C23C 26/00

(54) **COATED STEEL SHEET**

(30) Priority: 03.07.2023 JP 2023109649
(71) Applicant: Nippon Steel Corporation, Tokyo 100-8071 (JP)
(72) Inventor: KAWAMURA, Yasuaki, Tokyo 100-8071 (JP); FUJII, Takashi, Tokyo 100-8071 (JP); SHIBAO, Fumio, Tokyo 100-8071 (JP)
(74) Representative: Vossius & Partner Patentanwälte Rechtsanwälte mbB
(86) International application number: PCT/JP2024/024107
(87) International publication number: WO 2025/009563

(57) **Abstract**

[PROBLEM] To provide a painted steel sheet which can be further improved in corrosion resistance and productivity while having a low-gloss paint film layer having a particle or a thin film portion.

[SOLUTION] Provided is a painted steel sheet including two or more paint film layers including a rust preventive paint film layer on at least one side of a steel sheet having a Zn-containing plating layer, wherein: a 60-degree specular glossiness Gs (60°) specified in JIS Z 8741:1997 of the paint film layer on at least one face of the steel sheet is 20% or less; an average film thickness of the rust preventive paint film layer is 5 µm or more and 15 µm or less; the rust preventive paint film layer contains a binder resin, a cross-linking agent, and a rust preventive pigment; and in a cross section obtained by cutting the paint film layer in a thickness direction at an arbitrary position, a coverage ratio of the rust preventive pigment to a total area of the rust preventive paint film layer is 30% or more and 60% or less in terms of area ratio.

## Description

### TECHNICAL FIELD

The present invention relates to a painted steel sheet.

### BACKGROUND ART

Steel sheets with high design are increasingly used for applications for building material use, home appliance use, automobile use, and so on. A steel sheet has a matte appearance with suppressed gloss as an example of the high design. Examples of the steel sheet having the matte appearance include a low-gloss painted steel sheet with an organic coating layer containing resin particles which is provided on a steel sheet surface, and so on. Further, as a steel sheet having a paint film layer on the surface, there is a known steel sheet provided with a rust preventive paint film layer containing a rust preventive pigment for improving the corrosion resistance of the steel sheet.

For example, Patent Document 1 below proposes a technique of improving, in a zinc-based plated steel sheet having an organic coating, the abrasion resistance of the organic coating by containing a resin particle having a particle diameter larger than the film thickness of the organic coating (hereinafter, also referred to as a "large-diameter particle") in the organic coating.

### PRIOR ART DOCUMENT

### PATENT DOCUMENT

Patent Document 1: International Publication Pamphlet No. WO 2014/112544

### SUMMARY OF THE INVENTION

### PROBLEMS TO BE SOLVED BY THE INVENTION

The steel sheet having the matte appearance is subjected to low-gloss painting or the like and thus has large recesses and projections on a steel sheet surface to suppress the reflection of light by the recesses and projections and realize the low gloss. Accordingly, a layer constituting the low-gloss painting (hereinafter, also called a "low-gloss paint film layer") can contain a thin film portion. If a flaw or the like occurs at the thin film portion, a corrosion factor in an environment such as rain water is likely to intrude through the flaw or the like, and can be a factor causing corrosion on the steel sheet surface. Besides, if the organic coating containing the large-diameter particle as proposed in Patent Document 1 above is employed as the low-gloss paint film layer, the large-diameter particle is largely exposed from the binder resin layer constituting the organic coating. The corrosion factor is likely to intrude through the interface between the large-diameter particle and the binder resin layer, and can be a factor causing corrosion on the steel sheet surface.

Besides, if the zinc-based plated steel sheet having the organic coating containing the large-diameter particle is wound into a coil form or subjected to predetermined press processing, the large-diameter particle falls off the organic coating, resulting in a decrease in design of the organic coating in some cases. Further, the large-diameter particle that has fallen off the organic coating may contaminate various facilities for winding the steel sheet into the coil form or performing the press processing to hinder the processing. From the above, in the case of handling the organic coating containing the large-diameter particle, it is necessary to sufficiently pay attention on handling it and there is room for further improvement from the viewpoint of improving the productivity.

Hence, the present invention has been made in view of the above problems, and an object of the present invention is to provide a painted steel sheet which can be further improved in corrosion resistance and productivity while having a low-gloss paint film layer having a particle or a thin film portion.

### MEANS FOR SOLVING THE PROBLEMS

As a result of earnest studies for solving the above-described problems, the present inventors obtained the following findings. Specifically, if the surface of a particle having a particle diameter larger than an average film thickness contained in an organic resin coating layer can be covered by an organic resin, the interface between the large-diameter particle and the binder resin layer can be lengthened. Note that owing to the "interface between the large-diameter particle and the binder resin layer is long", a predetermined portion of the particle projecting from the binder resin layer is covered by a film-forming component, so that an exposed portion of the particle can be decreased. Further, lengthening the interface between the large-diameter particle and the binder resin layer as above can suppress the intrusion of the corrosion factor to suppress the corrosion. Further, it is possible to prevent the fall-off and deformation of the particle. Based on the idea, the present inventors discussed in detail coating conditions of a paint containing the particle having the particle diameter larger than the average film thickness. As a result of this, the present inventors have found that when the average particle diameter of the particle, the average film thickness of the organic resin coating layer, the thickness of the organic resin covering the surface of the particle, and so on satisfy specific conditions, it is possible to prevent the fall-off of the particle from the organic resin coating layer and deformation to further improve the design and the productivity of the painted steel sheet.

The gist of the present invention completed based on the above findings is as follows.
[1] A painted steel sheet including
   two or more paint film layers including a rust preventive paint film layer on at least one side of a steel sheet having a Zn-containing plating layer, wherein:
   a 60-degree specular glossiness Gs (60°) specified in JIS Z 8741:1997 of the paint film layer on at least one face of the steel sheet is 20% or less;
   an average film thickness of the rust preventive paint film layer is 5 µm or more and 15 µm or less;
   the rust preventive paint film layer contains a binder resin, a cross-linking agent, and a rust preventive pigment; and
   in a cross section obtained by cutting the paint film layer in a thickness direction at an arbitrary position, a coverage ratio of the rust preventive pigment to a total area of the rust preventive paint film layer is 30% or more and 60% or less in terms of area ratio.
[2] The painted steel sheet according to the above [1], wherein
   the rust preventive pigment contains at least one or more of Si, P, Mg, and V.
[3] The painted steel sheet according to the above [2], wherein
   the Si contains any one or more of calcium ion-exchanged silica and magnesium ion-exchanged silica, the P contains any one or more of zinc phosphate, magnesium dihydrogen phosphate, and aluminium dihydrogen triphosphate, and the Mg contains any one or more of magnesium dihydrogen phosphate, magnesium oxide, and magnesium hydroxide.
[4] The painted steel sheet according to the above [1] or [2], wherein:
   on the face of the steel sheet where the 60-degree specular glossiness Gs (60°) is 20% or less, the two or more paint film layers have the rust preventive paint film layer at a lower layer and have a colored paint film layer at an outermost layer located on a farthest side from the steel sheet, and the colored paint film layer contains a resin particle, and a binder resin, a cross-linking agent, and a color pigment as a film-forming component; and
   in the cross section, an average particle diameter of the resin particle is two times or more and five times or less an average film thickness at a portion not containing the resin particle of the outermost layer paint film layer.
   Where the average particle diameter is a value obtained by measuring, in one observation visual field region in the cross section, circle-equivalent diameters of the resin particles existing in the observation visual field region, calculating an average value of upper two circle-equivalent diameters in descending order of the circle-equivalent diameters, and further averaging the averaged values similarly obtained for the observation visual field regions at ten arbitrary locations, by a number of fields of view.
[5] The painted steel sheet according to the above [4], wherein
   the coverage ratio of the resin particles to a total area of the outermost layer paint film layer is 5% or more and 30% or less in terms of area ratio.
[6] The painted steel sheet according to the above [4], wherein
   in the cross section, a projecting portion of the resin particle projecting from a position on a surface at the portion not containing the resin particle of the outermost layer paint film layer is covered, at half or more of a length along an outer peripheral portion of the projecting portion, with the film-forming component having a thickness of 0.5 µm or more.
[7] The painted steel sheet according to the above [4], wherein
   the resin particle is a resin particle made of an acrylic resin.
[8] The painted steel sheet according to the above [5], wherein
   the resin particle is a resin particle made of an acrylic resin.
[9] The painted steel sheet according to the above [6], wherein
   the resin particle is a resin particle made of an acrylic resin.
[10] The painted steel sheet according to the above [4], wherein
   the binder resin is a binder resin made of an acrylic resin or a polyester resin.
[11] The painted steel sheet according to the above [5], wherein
   the binder resin is a binder resin made of an acrylic resin or a polyester resin.
[12] The painted steel sheet according to the above [6], wherein
   the binder resin is a binder resin made of an acrylic resin or a polyester resin.
[13] The painted steel sheet according to the above [7], wherein
   the binder resin is a binder resin made of an acrylic resin or a polyester resin.
[14] The painted steel sheet according to the above [8], wherein
   the binder resin is a binder resin made of an acrylic resin or a polyester resin.
[15] The painted steel sheet according to the above [9], wherein
   the binder resin is a binder resin made of an acrylic resin or a polyester resin.
[16] The painted steel sheet according to the above [1] or [2], having a characteristic selected from any one or two of a surface roughness of the steel sheet being 2 µm or more in Ra on the face of the steel sheet where the 60-degree specular glossiness Gs (60°) is 20% or less, and the paint film layer containing 15% or more of an aggregate composed of a pigment containing silica.

### EFFECT OF THE INVENTION

As explained above, according to the present invention, it becomes possible to prevent the fall-off of the particle from an organic resin coating layer and deformation to further improve the design and the productivity of a painted steel sheet.

### BRIEF DESCRIPTION OF THE DRAWINGS

FIG. 1A is a schematic view for explaining an example of a structure of a painted steel sheet according to an embodiment of the present invention.
FIG. 1B is a schematic view for explaining an example of a structure of a painted steel sheet according to the embodiment.
FIG. 1C is a schematic view for explaining an example of a structure of a painted steel sheet according to the embodiment.
FIG. 2A is a schematic view for explaining an outermost layer paint film layer in the painted steel sheet according to the embodiment.
FIG. 2B is a schematic view for explaining an outermost layer paint film layer in the painted steel sheet according to the embodiment.
FIG. 3A is a schematic view for explaining a thin film part in a painted steel sheet according to another embodiment.
FIG. 3B is a schematic view for explaining a thin film part in a painted steel sheet according to still another embodiment.

### EMBODIMENTS FOR CARRYING OUT INVENTION

Hereinafter, preferred embodiments of the present invention will be explained while referring to the accompanying drawings. Note that in the present description and the drawings, components having substantially the same functional configurations are denoted by the same reference numerals to omit overlapped explanation.

### [Regarding a steel sheet 10]

In a painted steel sheet 1 according to this embodiment, various types of steel sheets can be used as a steel sheet 10 being a base material. It is possible to use various types of steel sheets, as raw materials of the steel sheets, such as Al-killed steel, ultralow carbon steel containing Ti, Nb, and the like, high-strength steel further containing strengthening elements such as P, Si, and Mn in the ultralow carbon steel, and so on.

It is preferable to use, among the above various types of steel sheets, zinc-based plated steel sheets in which various types of zinc-based plating layers containing at least zinc are provided on surfaces of the steel sheets as substrates, as the steel sheet 10 according to this embodiment. Examples of the zinc-based plated steel sheets include zinc-based plated steel sheets such as a galvanized steel sheet, a zinc-nickel plated steel sheet, a zinc-iron plated steel sheet, a zinc-chromium plated steel sheet, a zinc-aluminum plated steel sheet, a zinc-titanium plated steel sheet, a zinc-magnesium plated steel sheet, a zinc-manganese plated steel sheet, a zinc-aluminum-magnesium plated steel sheet, and a zinc-aluminum-magnesium-silicon plated steel sheet. Further, as the zinc-based plated steel sheet, the ones containing cobalt, molybdenum, tungsten, nickel, titanium, chromium, aluminum, manganese, iron, magnesium, lead, bismuth, antimony, tin, copper, cadmium, arsenic, and the like as a small amount of dissimilar metal elements or impurities in the plating or the ones in which inorganic substances such as silica, alumina, titania, and the like are dispersed may be used. Further, as the zinc-based plated steel sheet, a steel sheet having multilayer plating made by combining the above plating and other type of plating (for example, iron plating, iron-phosphorus plating, nickel plating, cobalt plating, or the like) may be used. A plating method is not particularly limited and various known plating methods such as an electroplating method, a hot-dip plating method, a vapor deposition plating method, a dispersion plating method, a vacuum plating method, and so on may be used.

On the surface of the steel sheet 10, a paint film 11 is provided. The paint film 11 includes a rust preventive paint film layer 20. Further, in one embodiment, an outermost layer paint film layer 30 as a colored paint film layer according to this disclosure is included. In the paint film 11, the rust preventive paint film layer 20 is located on the surface of the steel sheet 10. Besides, the outermost layer paint film layer 30 is located at an outermost layer of the paint film 11. The paint film 11 according to this embodiment is provided such that the outermost layer paint film layer 30 is in contact with the surface of the rust preventive paint film layer 20, and another desired coating layer may be provided between the rust preventive paint film layer and the outermost layer paint film layer 30.

Here, the thickness of the above steel sheet 10 is not particularly limited, and may be appropriately set according to the mechanical strength (for example, tensile strength), workability, or the like required for the painted steel sheet 1 according to this embodiment.

### [Regarding the rust preventive paint film layer 20]

The rust preventive paint film layer 20 provided on the surface of the steel sheet 10 in the painted steel sheet 1 according to this embodiment will be explained. The rust preventive paint film layer 20 is a resin coating layer containing a binder resin, a cross-linking agent, and a rust preventive pigment.

The rust preventive paint film layer 20 is provided on one side (FIG. 1A) or both sides (FIGS. 1B, C) of the steel sheet 10 as illustrated in FIG. 1A to FIG. 1C. The provision on at least the one side of the steel sheet 10 can suppress the corrosion of the steel sheet 10 on that side. Further, the provision on both sides of the steel sheet 10 can suppress the corrosion of the steel sheet 10 on both sides and exhibit excellent end face corrosion resistance.

The binder resin contained in the rust preventive paint film layer 20 functions as a film-forming component, and any material can be used. However, from the viewpoints of ease of manufacturing and costs and the viewpoints of corrosion resistance and flaw resistance, it is preferable to use various types of organic resins as the resin. Examples of the resin include an acryl-based resin, a polyester-based resin, a urethane-based resin, a fluorine-based resin, and so on.

As the rust preventive pigment contained in the rust preventive paint film layer 20, various types of known rust preventive pigments containing a pigment containing at least one or more elements P, V, Si, and Mg can be used.

Examples of the pigment containing at least one or more elements P, V, Si, and Mg include the Si containing any one of calcium ion-exchanged silica and magnesium ion-exchanged silica, the P containing any one of zinc phosphate, magnesium dihydrogen phosphate, and aluminium dihydrogen triphosphate, the Mg containing any one of magnesium dihydrogen phosphate, magnesium oxide, and magnesium hydroxide, and the V containing calcium vanadate.

Besides, an average film thickness of the rust preventive paint film layer 20 is 5 µm or more and 15 µm or less. Setting the average film thickness of the rust preventive paint film layer 20 to 5 µm or more can achieve a sufficient effect of suppressing corrosion against a corrosion factor which can intrude through the interface between the thin film portion or particle and the binder resin. The average film thickness of the rust preventive paint film layer 20 is preferably 7.0 µm or more.

On the other hand, setting the average film thickness of the rust preventive paint film layer 20 to 15 µm or less can suppress the occurrence of a painting defect called popping during the paint baking. The average film thickness of the rust preventive paint film layer 20 is preferably 12 µm or less.

Further, the rust preventive paint film layer 20 has a coverage ratio of the rust preventive pigment to the total area of the rust preventive paint film layer 20 in observation of a cross section obtained by cutting the paint film 11 in a thickness direction at an arbitrary position is 30% or more and 60% or less in terms of area ratio. Setting the coverage ratio of the rust preventive pigment to 30% or more can achieve a sufficient effect of suppressing corrosion against a corrosion factor which can intrude through the interface between the thin film portion or particle and the binder resin. The coverage ratio of the rust preventive pigment is preferably 40% or more.

On the other hand, setting the coverage ratio of the rust preventive pigment to 60% or less can achieve sufficient adhesiveness between the rust preventive paint film layer 20 and the steel sheet 10, particularly, the adhesiveness at a worked portion. The coverage ratio of the rust preventive pigment is preferably 50% or less.

The average film thickness of the rust preventive paint film layer 20 can be specified by the following procedure. First, a cross section obtained by cutting the paint film 11 according to this embodiment in a thickness direction at an arbitrary position is focused on. Then, the cross section is observed under an electron microscope (more specifically, a field emission scanning electron microscope: FE-SEM). Next, the thickness of the rust preventive paint film layer 20 is measured at ten locations in a field of view in the focused cross section. In this event, the thickness of the rust preventive paint film layer 20 only needs to be measured using a length measurement function or the like installed in the FE-SEM. Then, an average value of obtained measured values at the ten locations is calculated, and regarded as an average value of the thicknesses of the rust preventive paint film layer 20 in the focused field of view. The above operation is performed for the fields of view at ten arbitrary locations, and average values obtained respectively from the fields of view are further averaged by the number of fields of view. The value obtained as above is regarded as an average film thickness of the rust preventive paint film layer 20.

Besides, the coverage ratio of the rust preventive pigment to the total area of the rust preventive paint film layer 20 is calculated as follows. Specifically, the cross section obtained by cutting the paint film 11 according to this embodiment in the thickness direction at the arbitrary position is focused on as with the measurement of the average film thickness. In the focused cross section, one observation visual field region (length in a width direction: 40 µm) is focused on. In this event, the magnification of the FE-SEM only needs to be set to an appropriate magnification (for example, about 3000 times) so that the length of 40 µm falls within one field of view in the width direction. Then, the area proportion (namely, the area ratio) of the rust preventive pigment to the total area of the rust preventive paint film layer 20 in the observation visual field region having the above size is calculated by various functions installed in the electron microscope, image processing, or the like. The above observation can be performed on the observation visual field regions at ten arbitrary locations to obtain ten measured values of the area ratio of the rust preventive pigment. An average value of the ten measured values thus obtained is calculated and regarded as an average area ratio of the rust preventive pigment in the cross section. As explained above, the average area ratio is an average value of the area proportion occupied by the rust preventive pigment to the total area of the rust preventive paint film layer 20 in the observation visual field regions at the ten locations observed. The average value is regarded as the coverage ratio of the rust preventive pigment. Note that the rust preventive pigment in the paint film 11 can be identified by confirming existing elements by an EDS analysis (Nergy Dispersive X-ray Spectroscopy) for the particles existing in the paint film 11.

### [Regarding the outermost layer paint film layer 30]

The outermost layer paint film layer 30 according to this embodiment is a resin coating layer which is located at the outermost layer of the paint film 11 as exemplified in FIG. 1A to FIG. 1C and has particles 101 existing in a dispersed state in a binder resin 103 as a film-forming component. The outermost layer paint film layer 30 may contain various additives such as a cross-linking agent, a coloring agent, and so on in addition to the above particles 101 and binder resin 103.

When a 60-degree specular glossiness Gs (60°) specified in JIS Z 8741:1997 is measured for the surface of the outermost layer paint film layer 30, a value of the 60-degree specular glossiness Gs (60°) is 20 or less. In the painted steel sheet 1 according to this embodiment, the surface of the outermost layer paint film layer 30 exhibits the glossiness in the above range, whereby the painted steel sheet 1 according to this embodiment exhibits a better matte appearance (eventually, better design). The value of the 60-degree specular glossiness Gs (60°) is more preferably 5 or more. Further, the value of the 60-degree specular glossiness Gs (60°) is more preferably 15 or less.

In the painted steel sheet 1 according to this embodiment, the particles 101 are dispersed in the binder resin 103 in the outermost layer paint film layer 30. In addition, the particles 101 satisfy the conditions explained in detail below. Thus, the binder resin 103 realizes predetermined corrosion resistance and flaw resistance. Further, the painted steel sheet 1 as a whole realizes excellent design having both a texture appearance and a matte appearance. Furthermore, lengthening the interface between the particle 101 and the binder resin 103 makes it possible to suppress the corrosion of the steel sheet. Secondarily, it becomes possible to prevent the generation of pressure marks due to relatively flattening of an organic coating at a deformed portion.

### <<Regarding the particle 101>>

In the outermost layer paint film layer 30 according to this embodiment, the particles 101 project from positions of the surface at portions not containing the particles 101 of the outermost layer paint film layer 30. This can realize the excellent design having both a texture appearance and a matte appearance as a whole of the painted steel sheet 1. The details of the relation between the outermost layer paint film layer 30 and the particles 101 will be explained later.

Further, the particles 101 preferably have predetermined toughness and expandability. The particles 101 having the predetermined toughness and expandability can mitigate the impact applied to the outermost layer paint film layer 30. As a result of this, in the painted steel sheet 1 according to this embodiment, the flaw resistance of the outermost layer paint film layer 30 can be further improved. Further, the particles 101 having the predetermined toughness and expandability can further prevent the generation of the pressure marks due to relatively flattening of the organic coating at the deformed portion. Furthermore, if the outermost layer paint film layer 30 is flawed, it is possible to prevent the flaw from reaching the steel sheet 10 and maintain the corrosion resistance of the painted steel sheet 1.

Here, in the outermost layer paint film layer 30 according to this embodiment, any particles made of various raw materials can be used as the particles 101 as long as they have the predetermined toughness and expandability. However, it is more preferable to use organic resin particles composed of an organic resin than inorganic particles composed of an inorganic resin represented by silica or ceramics from the viewpoint of having better toughness and expandability.

Examples of the organic resin particles to be used as the particles 101 include resin particles made of an acryl-based resin, resin particles made of a polyester-based resin, resin particles made of a urethane-based resin, resin particles made of a fluorine-based resin, resin particles made of a silicone resin, resin particles made of a polyolefin-based resin, and so on. It is more preferable to use, as the particles 101, the resin particles made of the urethane-based resin or the resin particles made of the acryl-based resin among them, from the viewpoint of more easily enabling the desired toughness and expandability. It is furthermore preferable to use, as the particles 101, resin particles using the acryl-based resin as a main component among them.

On the other hand, in the case of using particles of a thermoplastic resin as the resin particles, the particles preferably have a melting point at a level where they do not melt when a baking step is executed in a later-explained manufacturing process of the painted steel sheet. The particles 101 having the melting point can be made not to melt in the paint film baking step, resulting in the desired 60-degree specular glossiness Gs (60°). Though the baking will be explained later in detail, a peak metal temperature can be made to fall within a range of 180 to 250°C, and therefore the resin particles preferably have a melting point at a level exceeding the peak metal temperature.

Note that a plurality of types of particles having different average particle diameters may be contained as the particles 101. Further, the particles 101 may also have functions as various additives which can be added to the outermost layer paint film layer 30, such as the coloring agent, the rust preventive pigment, and so on.

### <<Regarding the binder resin 103>>

Besides, as the binder resin 103 as the film-forming component contained in the outermost layer paint film layer 30 according to this embodiment, any raw material can be used as long as it has the function as the binder for the particles 101. However, from the viewpoints of ease of manufacturing and costs and the viewpoints of corrosion resistance and flaw resistance, it is preferable to use various types of organic resins as the binder resin 103. Examples of the binder resin 103 include an acryl-based resin, a polyester-based resin, a urethane-based resin, a fluorine-based resin, and so on. It is more preferable to use a binder resin containing an acryl-based resin or a polyester-based resin as a main component among them.

Further, in a preferred embodiment of the outermost layer paint film layer 30, an organic resin high in affinity with the particles 101 is selected as the binder resin 103. This can further improve the affinity between the particles 101 and the binder resin 103 and further suppress the fall-off of the particles 101. Further, it is possible to further improve the adhesiveness and barrier property of the outermost layer paint film layer 30. As an example of the resin particle high in affinity with the particles 101, a resin of the same type as the particles 101 is selected. Further, in the case of selecting the acrylic resin as the particles 101 as another example of the resin particle high in affinity with the particles 101, a polyester-based resin is selected as the binder resin 103.

In the case of selecting the acrylic resin as the particles 101 in another preferred embodiment of the outermost layer paint film layer 30, a binder resin containing a polyester/melamine curable resin as a main component is selected as the binder resin 103. Thus, the affinity between the binder resin 103 and the acryl-based resin as the particles 101 can further improve owing to the action of the melamine resin as a cross-linking agent (curing agent) used for cross-linking (curing) of the binder resin 103 to further suppress the fall-off of the particles 101. In a preferred embodiment, the binder resin 103 is composed of a polyester/melamine curable resin.

### <Regarding the existing state of the particles 101 in the outermost layer paint film layer 30>

Next, a distribution state of the particles 101 in the outermost layer paint film layer 30 according to this embodiment will be explained in detail while referring to FIG. 2. FIG. 2 is an explanatory view for explaining the outermost layer paint film layer 30 in the painted steel sheet 1 according to this embodiment.

In the painted steel sheet 1 according to this embodiment, the particles 101 exist in a state of dispersing in the film-forming component such as the binder resin 103, the color pigment, and so on constituting the outermost layer paint film layer 30. For discussion of the existing state of the particles 101, a cross section obtained by cutting the paint film 11 according to this embodiment in a thickness direction at an arbitrary position is focused on as schematically illustrated in FIG. 2. Then, the cross section is observed under the FE-SEM and the existing state of the particles 101 will be discussed.

More specifically, a cross section obtained by cutting the paint film 11 according to this embodiment in a thickness direction at an arbitrary position is focused on, as with the above rust preventive paint film layer 20. In the focused cross section, a region having a length of 40 µm in a direction (hereinafter, also referred to as a width direction) perpendicular to the thickness direction is regarded as an observation visual field region in one-time microscope observation, and the observation visual field region is arbitrarily set at ten locations in the focused cross section. Then, based on obtained measured results at the ten locations, a feature amount representing the existing state of the particles 101 explained below will be calculated.

### ◊ The coverage ratio of the particles 101 in the cross section

The coverage ratio of the particles 101 in the above cross section in the outermost layer paint film layer 30 according to this embodiment falls within a range of 5% or more and 30% or less in average value of the area ratio (namely, an average area ratio) being an area proportion of the particles 101 in the outermost layer paint film layer 30.

Here, the average area ratio is calculated as follows. Specifically, one observation visual field region (length in the width direction: 100 µm) is focused on in the cross section to be focused on. In this event, the magnification of the FE-SEM only needs to be set to an appropriate magnification (for example, about 1000 times) so that the length of 100 µm falls within one field of view in the width direction. Then, the area proportion (namely, the area ratio) of the particles 101 in the outermost layer paint film layer 30 in the observation visual field region having the above size is calculated by various functions installed in the electron microscope, image processing, or the like. The above observation can be performed on the observation visual field regions at ten arbitrary locations to obtain ten measured values of the area ratio of the particles 101. An average value of the ten measured values thus obtained is calculated and regarded as an average area ratio of the particles 101 in the cross section. As explained above, the average area ratio is an average value of the area proportions occupied by the particles to the total area of the observation visual field regions at the ten locations observed.

When the average area ratio of the particles 101 in the cross section is less than 5%, the coverage proportion of the particles 101 is too small, it is impossible to realize the desired design. When the average area ratio of the particles 101 is 5% or more, it becomes possible to realize an excellent design having both a texture appearance and a matte appearance. The average area ratio of the particles 101 in the cross section is preferably 10% or more and more preferably 15% or more.

On the other hand, when the average area ratio of the particles 101 in the cross section is more than 30%, the coverage proportion of the particles 101 is too large, thereby not only failing to realize the flaw resistance required for the outermost layer paint film layer 30 but also failing to realize the desired design (specifically, the matte appearance). When the average area ratio of the particles 101 is 30% or less, it becomes possible to realize the desired design while realizing the flaw resistance required for the outermost layer paint film layer 30. The average area ratio of the particles 101 in the cross section is preferably 25% or less and more preferably 20% or less.

### ◊ An average film thickness T of the outermost layer paint film layer 30 at portions not containing the particles 101

The average film thickness T of the outermost layer paint film layer 30 at the portions not containing the particles 101 in the above cross section in the outermost layer paint film layer 30 according to this embodiment is preferably 10 µm or more. Further, the average film thickness T is preferably 40 µm or less. When the average film thickness T of the outermost layer paint film layer 30 at the portions not containing the particles 101 in the cross section is less than 10 µm, the thickness of the outermost layer paint film layer 30 is too small, failing to realize the desired corrosion resistance. When the average film thickness T is 10 µm or more, it becomes possible to realize the corrosion resistance required for the painted steel sheet 1 according to this embodiment. The average film thickness T is more preferably 12 µm or more and furthermore preferably 15 µm or more.

On the other hand, when the average film thickness T of the outermost layer paint film layer 30 at the portions not containing the particles 101 in the cross section is more than 40 µm, the thickness of the outermost layer paint film layer 30 is too large, resulting in an undesirable decrease in the adhesiveness of the outermost layer paint film layer 30. When the average film thickness T is 40 µm or less, it is possible to realize the desired corrosion resistance while maintaining the adhesiveness of the outermost layer paint film layer 30. The average film thickness T is preferably 35 µm or less and more preferably 25 µm or less.

Note that the average film thickness T of the outermost layer paint film layer 30 at the portions not containing the particles 101 in the above cross section is specified by the following procedure. First, the cross section obtained by cutting the paint film 11 according to this embodiment in the thickness direction at the arbitrary position is focused on, as with the above rust preventive paint film layer 20. The thickness of the outermost layer paint film layer 30 at the portion where the particle 101 does not exist is measured at least at ten or more locations in the one focused observation visual field region. In this event, the thickness of the outermost layer paint film layer 30 at the portion not containing the particle 101 only needs to be measured using the length measurement function installed in the FE-SEM. Then, an average value of the three or more obtained measured values is calculated, and regarded as an average value of the thicknesses of the outermost layer paint film layer 30 in the focused observation visual field region. The above operation is performed for the observation visual field regions at ten arbitrary locations, and average values obtained respectively from the observation visual field regions are further averaged by the number of fields of view. The value obtained as above is regarded as an average film thickness T of the outermost layer paint film layer 30 at the portions not containing the particles 101.

It is assumed that measured results of thicknesses T₁, T₂, and T₃ have been obtained respectively at three locations at the portions where the particles 101 do not exist as illustrated in FIG. 2 in the one focused observation visual field region. In this case, an average value of the thicknesses of the outermost layer paint film layer 30 in the one focused observation visual field region is (1/3) × (T₁ + T₂ + T₃). This observation is executed for the observation visual field regions at ten arbitrary locations, and a plurality of obtained average values are further averaged by the number of fields of view, whereby the average film thickness T of the outermost layer paint film layer 30 at the portions not containing the particles 101 is obtained.

### <<Regarding the existing state of the particles 101 in the outermost layer paint film layer 30>>

Next, an existing state of the particles 101 in the outermost layer paint film layer 30 will be explained in detail while referring to FIG. 2. FIG. 2 is a schematic view for explaining the particles 101 contained in the outermost layer paint film layer 30 in the painted steel sheet 1 according to this embodiment.

In the outermost layer paint film layer 30 according to this embodiment, an average particle diameter φ₁₀ of the particles 101 specified by the procedure explained later (hereinafter, simply referred to as an "average particle diameter φ₁₀") is two times or more and five times or less the average film thickness T at the portions not containing the particles 101 of the outermost layer paint film layer 30 (hereinafter, simply referred to as an "average film thickness T"). The painted steel sheet 1 containing the particles 101 having the relation between the average particle diameter φ₁₀ and the average film thickness T can realize the excellent design having both a texture appearance and a matte appearance as a whole. The particle 101 has an average particle diameter φ₁₀ of the particles 101 that is preferably 2.1 times or more, more preferably 2.2 times or more, more preferably 2.3 times or more, more preferably 2.4 times or more, and most preferably 2.5 times or more the average film thickness T of the outermost layer paint film layer 30. Further, the particle 101 has an average particle diameter φ₁₀ of the particles 101 that is preferably 4.5 times or less, more preferably 4 times or less, and most preferably 3.5 times or less the average film thickness T of the outermost layer paint film layer 30.

The above average particle diameter φ₁₀ of the particles 101 in the cross section is specified by the following procedure. First, the cross section obtained by cutting the paint film 11 according to this embodiment in the thickness direction at the arbitrary position is focused on, as with the above rust preventive paint film layer 20. In the one focused observation visual field region, circle-equivalent diameters of the particles 101 are measured as measured values to be used for calculating the average particle diameter φ₁₀ of the particles 101 existing in the region, and an average value of upper two circle-equivalent diameters in descending order of the circle-equivalent diameters of the particles 101 is calculated. This measurement is executed for the observation visual field regions at ten arbitrary locations, and average values respectively obtained from the observation visual field regions are further averaged by the number of fields of view. The thus-obtained value is regarded as the average particle diameter φ₁₀ of the particles 101.

### ◊ A projecting portion peripheral length L₁ and a particle covered portion length L₂ in the cross section

Further, in the cross section obtained by cutting the paint film 11 in the thickness direction at the arbitrary position, a projecting portion of the particle 101 projecting from a position on the surface at the portion not containing the particle 101 of the outermost layer paint film layer 30 (hereinafter, referred to as a "projecting portion P") is covered, at half or more of a length along an outer peripheral portion of the projecting portion (hereinafter, referred to as a "projecting portion peripheral length L₁"), with the film-forming component having a thickness of 0.5 µm or more.

In the example illustrated in FIG. 2, a portion located above a segment B of a dotted line obtained by linking positions of the surface of the outermost layer paint film layer 30 at portions where the particles 101 do not exist is the projecting portion P. Besides, a portion of the particle 101 covered with the film-forming component having a thickness of 0.5 µm or more of the projecting portion P is called a "particle covered portion C" and a portion of the particle 101 not covered with the film-forming component having a thickness of 0.5 µm or more is called a "particle exposed portion E". The above "projecting portion P of the particle 101 is covered, at half or more of a length along an outer peripheral portion of the projecting portion P, with the film-forming component" means, in other words, that a ratio (L₂/L₁) of the length of the particle covered portion C along the outer peripheral portion of the projecting portion P (hereinafter, referred to as a "particle covered portion peripheral length L₂") to the projecting portion peripheral length L₁ is 1/2 or more. Note that all the projecting portion P may be covered with the film-forming component, as the particle 101 illustrated on the right side in FIG. 2. In this case, the projecting portion peripheral length L₁ and the particle covered portion peripheral length L₂ are equal, and the above ratio (L₂/L₁) is 1.

In the outermost layer paint film layer 30 according to this embodiment, half or more of the projecting portion P of the particle 101 is covered with the film-forming component, so that the interface between the particle 101 and the film-forming component can be lengthened. Therefore, in the painted steel sheet 1 according to this embodiment, it is possible to suppress the intrusion of a corrosion factor from the interface and to suppress the corrosion on the surface of the steel sheet 10. From these viewpoints, the ratio (L₂/L₁) between the projecting portion peripheral length L₁ and the particle covered portion peripheral length L₂ is preferably 3/5 or more.

The projecting portion peripheral length L₁ and the particle covered portion peripheral length L₂ in the cross section are specified by the following procedure. First, the cross section obtained by cutting the paint film 11 according to this embodiment in the thickness direction at the arbitrary position is focused on, as with the above rust preventive paint film layer 20. All of the particles 101 each having the particle exposed portion E are specified in the visual field in the focused cross section. Here, it is clear that the particle 101 not having the particle exposed portion E (for example, the particle 101 on the right side in FIG. 2) has the above ratio (L₂/L₁) of 1 because the projecting portion peripheral length L₁ and the particle covered portion peripheral length L₂ are equal, and therefore the measurement therefore is omitted. For each of the specified particles 101 each having the particle exposed portion E, the line segment B of the dotted line obtained by linking positions of the surface of the outermost layer paint film layer 30 at portions where the particles 101 do not exist is defined. The length of an arc linking two intersection points between the line segment B and the outer periphery of the particle 101 is measured and regarded as the projecting portion peripheral length L₁. Further, a length L₂₁ of an arc linking a left one of the two intersection points between the line segment B and the outer periphery of the particle 101 and a left one of two points on the outer periphery of the particle 101 at the boundary between the particle covered portion C and the particle exposed portion E, and a length L₂₂ of an arc linking a right one of the two intersection points between the line segment B and the outer periphery of the particle 101 and a right one of the two points on the outer periphery of the particle 101 at the boundary between the particle covered portion C and the particle exposed portion E are measured, and a length obtained by adding the lengths L₂₁ and L₂₂ of the arc is regarded as the particle covered portion peripheral length L₂. The projecting portion peripheral length L₁ and the lengths L₂₁ and L₂₂ of the arc can be calculated by various functions installed in the electron microscope, image processing, or the like. Further, the above ratio (L₂/L₁) is calculated. When the above ratio (L₂/L₁) calculated in this manner for each of the particles 101 is 1/2 or more, it can be said that "the projecting portion P of the particle 101 is covered, at half or more of a length along an outer peripheral portion of the projecting portion P, with the film-forming component". Note that a point G in FIG. 2 is the center of gravity of the particle 101.

Note that a percentage of the particles 101 each having the above ratio (L₂/L₁) between the projecting portion peripheral length L₁ and the particle covered portion peripheral length L₂ of 1/2 or more is most preferably 100%. However, it is considered that the one whose particle exposed portion E is expanded due to the use state or the one exceptionally having the above ratio (L₂/L₁) outside the above prescribed range may be contained. Therefore, the percentage of the particles 101 each having the above ratio (L₂/L₁) between the projecting portion peripheral length L₁ and the particle covered portion peripheral length L₂ of 1/2 or more may be 60% or more, and more preferably 80% or more.

### ◊ An average particle diameter of all of the particles 101

The average particle diameter φ₁₀ of the particles 101 has the above configuration, and the average particle diameter of all of the particles 101 is preferably 15 µm or more when the film thickness of the rust-proof paint film is 10 µm. Further, the average particle diameter of all of the particles 101 is preferably 40 µm or less when the film thickness of the rust-proof paint film is 10 µm. When the average particle diameter of all of the particles 101 is less than 15 µm, the average particle diameter of the particles 101 is too small, failing to realize the desired design and flaw resistance. When the average particle diameter of all of the particles 101 is 15 µm or more, it is possible to realize the design and flaw resistance required for the painted steel sheet 1 according to this embodiment. The average particle diameter of the particles 101 is more preferably 18 µm or more, and furthermore preferably 20 µm or more.

On the other hand, when the average particle diameter of the particles 101 is more than 40 µm, the average particle diameter of the particles 101 is too large, possibly resulting in a lack or the like of the particles in the manufacturing process. When the average particle diameter of the particles 101 is 40 µm or less, it is possible to suppress a lack of particles and realize stable manufacturing. The average particle diameter of the particles 101 is more preferably 30 µm or less.

The average particle diameter of all of the particles 101 can be measured as with the average particle diameter φ₁₀ of upper ten particles 101. Specifically, in the one observation visual field when calculating the average particle diameter φ₁₀, the average value of the circle-equivalent diameters of all of the particles 101 in the observation visual field is calculated. This measurement is executed for the observation visual field regions at ten arbitrary locations, and average values obtained respectively from the observation visual field regions are further averaged by the number of fields of view. The thus-obtained value is regarded as the average particle diameter of all of the particles 101.

### ◊ A ratio between a minimum film thickness and a maximum film thickness of the outermost layer paint film layer 30

In the outermost layer paint film layer 30 according to this embodiment, a ratio (H_{MAX}/Hₘᵢₙ) of a maximum film thickness H_{MAX} to a minimum film thickness Hₘᵢₙ specified by the following procedure is preferably 5 or more and 20 or less. When the ratio (H_{MAX}/Hₘᵢₙ) is within the above range, the value of the 60-degree specular glossiness Gs (60°) of the outermost layer paint film layer 30 can be made more preferable one. This exhibits a better matte appearance (eventually, a better design). Further, when the ratio (H_{MAX}/Hₘᵢₙ) is set to 5 or more, the tactile impression of the surface of the painted steel sheet 1 can be more preferable. From the viewpoint, the ratio (H_{MAX}/Hₘᵢₙ) of the maximum film thickness H_{MAX} is more preferably 6 or more, and furthermore preferably 7.5 or more. Further, the ratio (H_{MAX}/Hₘᵢₙ) is more preferably 17.5 or less, and furthermore preferably 15 or less.

Besides, when the ratio (H_{MAX}/Hₘᵢₙ) is within the above range, a portion of the minimum film thickness Hₘᵢₙ in the outermost layer paint film layer 30 may be a thin film portion. In this case, when a flaw or the like occurs at the thin film portion, a corrosion factor is likely to intrude through the flaw. In contrast to this, in the painted steel sheet 1 according to this embodiment, the rust preventive paint film layer 20 is provided and thus can suppress the corrosion on the surface of the steel sheet 10 even if the corrosion factor intrudes.

The ratio (H_{MAX}/Hₘᵢₙ) of the maximum film thickness H_{MAX} to the minimum film thickness Hₘᵢₙ is specified by the following procedure. First, the cross section obtained by cutting the paint film 11 according to this embodiment in the thickness direction at the arbitrary position is focused on, as with the above rust preventive paint film layer 20. In the one focused observation visual field region, a portion of a local minimum film thickness hₘᵢₙ and a portion of a local maximum film thickness h_{MAX} are specified using, for example, the length measurement function installed in the FE-SEM or the like, and their film thicknesses are measured. The above operation is performed for the observation visual field regions at ten arbitrary locations. Then, a smallest value among the local minimum film thicknesses hₘᵢₙ obtained respectively from the observation visual field regions is regarded as the minimum film thickness Hₘᵢₙ and a largest value among the local maximum film thicknesses h_{MAX} is regarded as the maximum film thickness H_{MAX}. Further, the ratio (H_{MAX}/Hₘᵢₙ) of the maximum film thickness H_{MAX} to the minimum film thickness Hₘᵢₙ is specified from the obtained values.

Here, as exemplified in FIG. 2B, the portion of the local minimum film thickness hₘᵢₙ is a portion where the outermost layer is thinnest in each visual field, that is, a portion where the distance between a surface on a side in contact with the rust preventive paint film layer 20 and an exposed surface S is shortest. Besides, a portion of the local maximum film thickness h_{MAX} is a portion where the film thickness of the outermost layer paint film layer 30 is largest in each visual field, that is, a portion where the distance between a surface on a side in contact with the rust preventive paint film layer 20 and the exposed surface S is largest. However, the above "distance" is in a direction perpendicular to the in-plane direction of the steel sheet 10.

Note the "exposed surface S" in the outermost layer paint film layer 30 includes an exposed surface Sa of the binder resin 103 at the portion where the particle 101 does not exist, an exposed surface Sb of the particle exposed portion E of the particle 101, and an exposed surface Sc of the binder resin 103 at the particle covered portion C. For example, portions of h₁ to h₄ indicating the film thicknesses of the outermost layer paint film layer 30 as illustrated in FIG. 2B are considered. In this case, at the portions of the film thickness h₁ and the film thickness h₃, the distances between the surface on the side in contact with the rust preventive paint film layer 20 and the exposed surface Sa of the binder resin 103 at the portions where the particles 101 do not exist are the thicknesses h₁, h₃, respectively. Besides, at the portion of the film thickness h₂, the distance between the surface on the side in contact with the rust preventive paint film layer 20 and the exposed surface Sb at the particle exposed portion E is the thickness h₂. Besides, at the portion of the film thickness h₄, the distance between the surface on the side in contact with the rust preventive paint film layer 20 and the exposed surface Sc of the binder resin 103 at the particle covered portion C is the thickness h₄.

For specifying the local minimum film thickness hₘᵢₙ and the local maximum film thickness h_{MAX} in the example of FIG. 2B, the largest one of the film thicknesses h₁ to h₄ is h₂, and therefore this portion is specified as the portion of the local maximum film thickness H_{MAX}. Besides, the smallest one is h₃, and therefore this portion is specified as the portion of the local minimum film thickness hₘᵢₙ. In the observation of the cross section, the local minimum film thickness hₘᵢₙ and the local maximum film thickness h_{MAX} are specified in the above manner.

### <<Regarding another configuration of the outermost layer paint film layer 30>>

The outermost layer paint film layer 30 can take another desired configuration not containing the particles 101 as long as the value of the 60-degree specular glossiness Gs (60°) of the outermost layer paint film layer 30 is 20% or less.

In one embodiment, the outermost layer paint film layer 30 can include a thin film part 200 in the observation of the cross section obtained by cutting the paint film 11 in the thickness direction at the arbitrary position. FIG. 3A and FIG. 3B are cross-sectional views illustrating the configuration of the painted steel sheet 1 including the outermost layer paint film layer 30 including the thin film part 200. When a flaw or the like occurs in the thin film part 200, a corrosion factor is likely to intrude through the flaw. In contrast to this, in the painted steel sheet 1 according to this embodiment, the rust preventive paint film layer 20 is provided and therefore can suppress the corrosion at the surface of the steel sheet 10 even if the corrosion factor intrudes.

Regarding the thin film part 200, in the example of FIG. 3A, when the upper surface of the steel sheet 10 is a flat shape and the upper surface of the outermost layer paint film layer 30 is a rough surface shape having certain recesses and projections, a portion between the painted steel sheet 1 and a recess of the outermost layer paint film layer 30 corresponds to the thin film part 200. The thin film part 200 in this case is 20 µm or less as an example. An example of the conceivable case that the outermost layer paint film layer 30 has a rough surface shape having the certain recesses and projections is a case where the outermost layer paint film layer 30 contains 1% or more of a curing catalyst and the outermost layer paint film layer 30 thus cures and shrinks to have the recesses and projections.

Besides, in the example of FIG. 3B as another example, when the upper surface of the steel sheet 10 has a rough surface shape having certain recesses and projections and the upper surface of the outermost layer paint film layer 30 has a flat shape, a portion between a projection of the painted steel sheet 1 and the outermost layer paint film layer 30 may correspond to the thin film part 200. The thin film part 200 in this case is 20 µm or less as an example. An example of the conceivable case that the painted steel sheet 1 has a rough surface shape having the certain recesses and projections is a case where the surface roughness of the painted steel sheet 1 is 2 µm or more in Ra.

### (Regarding the manufacturing method of the painted steel sheet)

Next, an example of the manufacturing method of the painted steel sheet according to this embodiment will be explained.

First, various pre-treatments including an alkali degreasing treatment, a washing treatment, a pickling treatment, and so on are performed on the steel sheet being the base material to make a clean steel sheet surface.

Then, various known rust preventive paints for forming a rust preventive paint film layer are applied to the steel sheet and dried. Here, the application of the above rust preventive paint can be performed by generally known coating methods such as roll coating, curtain flow coating, air spraying, airless spraying, immersion, bar coating, brushing, and the like. Besides, the heating method of the rust preventive paint is not particularly limited and, for example, any method such as hot air, near-infrared ray, far-infrared ray, induction heating, and a heating method by combination of them may be employed.

Next, a coating solution for forming an organic resin coating layer to the surface of the steel sheet formed with the rust preventive paint film layer and dried by heating to form the organic resin coating layer. Here, the coating solution is prepared by incorporating the above binder resin and various additives as necessary into a solvent. The above particles may be incorporated in the coating solution to be applied to at least one surface of the steel sheet as necessary to form the outermost layer paint film layer 30. Further, as necessary, a coating solution for forming another organic resin coating layer may be applied to the surface of the rust preventive paint film layer to form an outermost layer paint film layer on the surface of the other organic resin coating layer.

Besides, it is important to perform the application of the prepared coating solution using a curtain flow coater. By applying the coating solution containing particles using the curtain flow coater, it is possible to apply the coating solution without precipitating particles or causing paint defect (roping).

After the coating solution is applied to the surface of the rust preventive paint film layer, baking of heat-curing the coating solution is performed. In the baking, the heating temperature may be set according to the solvent to be used and is preferably set to, for example, a range of 180 to 250°C as a peak metal temperature. Further, when heat-curing the coating solution, it is necessary to pay attention to a temperature increasing rate. More specifically, it is important to set the temperature increasing rate to a range of 5 to 50 °C/sec. By applying the coating solution having the above surface tension and viscosity by the curtain flow coater and heat-curing it under a situation of the above temperature increasing rate, the organic resin coating layer in which the above-explained state of the particles is realized can be formed. The temperature increasing rate is more preferably in a range of 10 to 30 °C/sec.

Note that the heating method of the coating solution is not particularly limited but, for example, any method such as hot air, near-infrared ray, far-infrared ray, induction heating, and a heating method by a combination of them may be employed.

The manufacturing method of the painted steel sheet according to this embodiment has been explained above.

### EXAMPLES

Hereinafter, the painted steel sheet according to this embodiment will be concretely explained with examples and comparative examples. Note that the following examples are merely examples of the painted steel sheet according to this embodiment and the painted steel sheet according to this embodiment is not limited to the following examples.

### (1) Steel sheet

Five types of steel sheets of A1 to A5 listed in Table 1 below were prepared (all of them are commercially available). The plating weight is a weight per one side in Table 1 below. For the prepared steel sheets, a plated steel sheet (sheet thickness of 0.6 mm) made by performing a chromate-free-based paint base treatment (equivalent to CT-E300/Nippon Parkerizing Co., Ltd.) of 60 mg/m² was also prepared. A treatment solution used for the paint base treatment contains a silane coupling agent as its component, and a coating layer formed by the paint base treatment functions as a paint base treatment coating layer. Note that the presence or absence of the paint base treatment is listed in Tables 4-1 to 4-3 below.

### (2) Rust preventive paint film layer

First, clear rust preventive paints B1 to B3 below containing no rust preventive pigment were prepared by the following procedure. Then, any one or two or more of rust preventive pigments C1 to C5 listed in Table 2 were added and subjected to pigment dispersion to produce rust preventive paints. In the case of using the clear rust preventive paint B1, the polyester resin and the epoxy resin contained therein mainly function as the binder resin in the rust preventive paint film layer. In the case of using the clear rust preventive paint B2, the polyester resin contained therein mainly functions as the binder resin in the rust preventive paint film layer. In the case of using the clear rust preventive paint B3, the polyester resin and the urethane resin contained therein mainly function as the binder resin in the rust preventive paint film layer. After the produced rust preventive paints were used and applied to the one side of the steel sheet subjected to the base treatment by a bar coater, and then baked at a PMT (steel sheet peak metal temperature) of 220°C±10°C and for a baking time of 10 seconds. The types and the coverage ratios (%) of the rust preventive pigments C1 to C5 of the produced rust preventive paint films and the total coverage ratio (%) obtained by adding the coverage ratios of all contained rust preventive pigments are listed in Tables 4-1 to 4-3. Further, the film thickness (µm) of the rust preventive paint film is listed in Tables 4-1 to 4-3. In Table 2, "SHIELDEX" is a registered trademark, "K-WHITE" is a registered trademark, and "Kyowamag" is a registered trademark.

### <Clear rust preventive paint: B1>

It was produced by blending a polyester resin (VYLON TM270 manufactured by TOYOBO. CO., LTD, "VYLON" is a registered trademark), an epoxy resin (EPICLON TM1000 manufactured by DIC, "EPICLON" is a registered trademark), and a melamine resin as a cross-linking agent (CYMEL 327 manufactured by allnex, "CYMEL" is a registered trademark) at a solid content ratio of 75:5:20 and adding an organic solvent (using a mixture of cyclohexanone:Solvesso 150 = 1:1 in mass ratio) so that a solid content concentration was 25 mass% for adjustment.

### <Clear rust preventive paint: B2>

It was produced by blending a polyester resin (VYLON GK-140 manufactured by TOYOBO. CO., LTD) and a melamine resin as a cross-linking agent (CYMEL 327 manufactured by allnex) at a solid content ratio of 80:20 and adding an organic solvent (using a mixture of cyclohexanone: Solvesso 150 = 1:1 in mass ratio) so that a solid content concentration was 25 mass% for adjustment.

### <Clear rust preventive paint: B3>

It was produced by blending a polyester resin (VYLONAL MD1480 manufactured by TOYOBO. CO., LTD, "VYLONAL" is a registered trademark), a urethane resin (SUPERFLEX 150 manufactured by DKS Co. Ltd., "SUPERFLEX" is a registered trademark), and a melamine resin as a cross-linking agent (CYMEL 327 manufactured by allnex) at a solid content ratio of 40:40:20 and adding water so that a solid content concentration was 25 mass% for adjustment.

### (3) Outermost layer paint film layer

A paint used as the outermost layer paint film was "FLC 100 HQ (white type)" manufactured by Nippon Paint Co., Ltd. being a commercially available polyester-based overcoat coating paint as the binder resin. The outermost layer paint film was produced by adding a predetermined amount of any one or two or more of resin particles D1 to D10, D13, or D14 listed in Table 3, silica D11 as an aggregate, and a curing catalyst D12 to the paint for adjustment. Note that the viscosity was adjusted by adding an organic solvent (using a mixture of cyclohexanone:Solvesso 150 = 1:1 in mass ratio) according to the viscosity of the produced paint. The produced paint was used and applied to the one side of the steel sheet applied with the rust preventive paint film by a curtain coater or a bar coater. In the case of the curtain coater, after the application by the curtain coater, baking was performed at a PMT (steel sheet peak metal temperature) of 230°C and for a baking time of 40 seconds. Also in the case of the bar coater, baking was similarly performed at a PMT (steel sheet peak metal temperature) of 230°C and for a baking time of 12 seconds. In some samples, the baking was performed with the baking time changed while keeping the PMT at 230°C. The coating methods used are listed in Table 5-1 to Table 5-3. The rust preventive paint film and the outermost layer paint film were applied only on the front surface, or both of the front surface and the rear surface. The presence or absence and the type of the coating film on the rear surface are listed in Table 5. In Table 3, "GRANPEARL" is a registered trademark and "Sylosphere" is a registered trademark.

A resin particle coverage ratio (%) of each of the produced outermost layer paint film layers and a total coverage ratio (%) obtained by adding all of the contained resin particles are listed in Table 5-1 to Table 5-3. Further, the film thickness T (µm) of the outermost layer paint film and the ratio (particle diameter/film thickness) between the average particle diameter φ₁₀ and the average film thickness T are listed in Table 5-1 to Table 5-3. Further, in Table 5-1 to Table 5-3, the one having a percentage of the above ratio (L₂/L₁) between the projecting portion peripheral length L₁ and the particle covered portion peripheral length L₂ in each resin particle of 1/2 or more of 60% or more is indicated with "o" as being excellent in resin particle coverage, and the one having the percentage of less than 60% is indicated with "×" as not being excellent in resin particle coverage. Further, the ratio of the maximum film thickness to the minimum film thickness of the outermost layer paint film layer (maximum film thickness/minimum film thickness) is listed in Table 5-1 to Table 5-3.

For each of the obtained sample materials, the glossiness (more specifically, the 60-degree specular glossiness Gs (60°)) was measured according to the above-explained method, and is listed in Table 6-1 to Table 6-3 below.

Further, the corrosion resistance (corrosion resistance 1), the end face corrosion resistance (corrosion resistance 2), and so on on the paint film formation surface were measured. Further, the flaw resistance on the paint film formation surface was evaluated. The obtained results are collectively listed in Table 6-1 to Table 6-3 below. The evaluation method is as follows.

### (Corrosion resistance 1)

For the corrosion resistance (corrosion resistance 1) on the paint film formation surface, the end face of the surface treated steel sheet was sealed with tape, a cross cut reaching a steel sheet base material was applied to a test piece central portion with a cutter, and then an average paint film blister width from a cut part after execution of a salt spray (SST, 5% NaCl, 35° atmosphere) for 500 hr was measured and calculated. Note that the average paint film blister width can be calculated by measuring the area of a paint film blister part and then dividing it by a cut part length. Further, evaluation criteria are as follows. The acceptable level was set to 3 or higher.

### <Evaluation criteria>

Grade 5: less than 0.5 mm and no red rust generation
4: 0.5 mm or more and less than 1 mm and no red rust generation
3: 1 mm or more and less than 2 mm and no red rust generation
2: 2 mm or more and less than 5 mm and no red rust generation
1: 5 mm or more or red rust generation

### (Corrosion resistance 2)

For the end face corrosion resistance (corrosion resistance 2), the upper and lower end faces of the surface treated steel sheet were sealed with tape in a sample material having the rust preventive paint film and the outermost layer paint film formed on both the front surface and the rear surface, and then average paint film blister widths from right and left end face portions (left: lower burr, right: upper burr) after execution of a salt spray (SST, 5% NaCl, 35° atmosphere) for 500 hr were measured and calculated. Note that the average paint film blister width can be calculated by measuring the area of a paint film blister part and then dividing it by an end face part length. Further, evaluation criteria are as follows. The acceptable level was set to 2.

### <Evaluation criteria>

Grade 2: average blister width of less than 5 mm and no red rust generation
1: average blister width of 5 mm or more or red rust generation

### (Flaw resistance)

For the flaw resistance on the paint film formation surface, the flaw resistance was evaluated by a coin scratch test. A coin was brought into contact, in a state of being inclined at 45 degrees, with the painted surface of a produced sample, and scratched it with a load of 500 g. An applied flaw was evaluated on the basis of the following criteria, and the acceptable level was set to 3 or higher.

### <Evaluation criteria>

Grade 4: No paint film peeling or very slight paint film peeling is observed.
3: Slight paint film peeling is observed.
2: Partial paint film peeling is observed.
1: Paint film is completely peeled.

### (Roughness measurement)

A roughness (arithmetic mean roughness Ra) obtained from the surface of the painted steel sheet was obtained by a contact-type roughness gauge compliant with JIS B 0601: 2001. The measured length was set to 8.0 mm and the cutoff value was set to 0.8 mm. Ra of 2 µm or more was regarded as ∘ and Ra of less than 2 µm was regarded as ×.

### (Fall-off inspection of the particle)

A sample containing the resin particles in the outermost layer paint film layer was subjected to cylindrical drawing (drawing conditions: blank diameter of 100 mmφ, punch diameter of 50 mmφ, die diameter of 52.4 mmφ, and blank holder force (BHF) of 1.5 ton) so that a test surface (painted surface) was the outer surface, and then the presence or absence of flaw generation on the cylindrical drawn wall surface was visually confirmed. Regarding a flaw generation site where the flaw generation was confirmed, a wall portion including a flaw portion was cut out and confirmed whether the fall-off of the resin particles occurred by the surface SEM observation. The one in which the flaw generation on the wall portion was not confirmed or the one in which the flaw generation was confirmed but the fall-off of the resin particles did not occur was regarded as ∘, and the one in which the flaw generation was confirmed and the occurrence of the fall-off of the resin particles was confirmed was regarded as ×.

### [Table 1]

**TABLE 1**

| TYPE | METAL SHEET (HEREINAFTER, % REPRESENTS MASS%) |
|---|---|
| A1 | HOT-DIP GALVANIZED STEEL SHEET (PLATING WEIGHT 60 g/m2 ON ONE SIDE) |
| A2 | ALLOYED HOT-DIP GALVANIZED STEEL SHEET (Fe: 10%) (PLATING WEIGHT 50 g/m2 ON ONE SIDE) |
| A3 | HOT-DIP Al-9% Si PLATED SHEET SHEET (PLATING WEIGHT 60 g/m2 ON ONE SIDE) |
| A4 | HOT-DIP Zn-11% Al-3% Mg-0.2% Si PLATED SHEET SHEET (PLATING WEIGHT 100 g/m2 ON ONE SIDE) |
| A5 | STEEL SHEET (WITHOUT PLATING) |

### [Table 2]

**TABLE 2**

| TYPE | RUST PREVENTIVE PIGMENT |
|---|---|
| C1 | Ca ION-EXCHANGED SILICA "SHIELDEX C303" MANUFACTURED BY GRACE INC., CONTAINING Si |
| C2 | ALUMINIUM DIHYDROGEN TRIPHOSPHATE SUBJECTED TO Mg TREATMENT "K-WHITE G105" MANUFACTURED BY TAYCA CORPORATION, CONTAINING Mg, P |
| C3 | ALUMINIUM DIHYDROGEN TRIPHOSPHATE "K-WHITE #82" MANUFACTURED BY TAYCA CORPORATION, CONTAINING P |
| C4 | MAGNESIUM OXIDE "KYOWAMAG MF-30" MANUFACTURED BY KYOWA CHEMICAL INDUSTRY CO .,LTD., CONTAINING Mg |
| C5 | CALCIUM VANADATE GENERAL REAGENT CONTAINING V |

**[Table 3]**

| TYPE | | RESIN PARTICLE, AGGREGATE, OR CURING CATALYST |
|---|---|---|
| D1 | RESIN PARTICLE | "MX-150" (ACRYLIC RESIN PARTICLE, AVERAGE PARTICLE DIAMETER 1.5 µm) MANUFACTURED BY SOKEN CHEMICAL ENGINEERING CO., LTD. |
| D2 | RESIN PARTICLE | "MX-300" (ACRYLIC RESIN PARTICLE, AVERAGE PARTICLE DIAMETER 3 µm) MANUFACTURED BY SOKEN CHEMICAL ENGINEERING CO., LTD. |
| D3 | RESIN PARTICLE | "MX-500L" (ACRYLIC RESIN PARTICLE, AVERAGE PARTICLE DIAMETER 5 µm) MANUFACTURED BY SOKEN CHEMICAL ENGINEERING CO., LTD. |
| D4 | RESIN PARTICLE | "MX-1000" (ACRYLIC RESIN PARTICLE, AVERAGE PARTICLE DIAMETER 10 µm) MANUFACTURED BY SOKEN CHEMICAL 6 ENGINEERING CO., LTD. |
| D5 | RESIN PARTICLE | "MX-2000" (ACRYLIC RESIN PARTICLE, AVERAGE PARTICLE DIAMETER 20 µm) MANUFACTURED BY SOKEN CHEMICAL ENGINEERING CO., LTD. |
| D6 | RESIN PARTICLE | "MX-3000" (ACRYLIC RESIN PARTICLE, AVERAGE PARTICLE DIAMETER 30 µm) MANUFACTURED BY SOKEN CHEMICAL ENGINEERING CO., LTD. |
| D7 | RESIN PARTICLE | "GRANPEARL GU-0700P" (URETHANE RESIN-BASED PARTICLE, AVERAGE PARTICLE DIAMETER 7 µm) MANUFACTURED BY AICA KOGYO COMPANY, LIMITED |
| D8 | RESIN PARTICLE | "GRANPEARL GU-2000P" (URETHANE RESIN-BASED PARTICLE, AVERAGE PARTICLE DIAMETER 20 µm) MANUFACTURED BY AICA KOGYO COMPANY, LIMITED |
| D9 | RESIN PARTICLE | "FLOW BEAD CL-2080" (POLYETHILENE PARTICLE (MELTING POINT 105°C, AVERAGE PARTICLE DIAMETER 11 µm)) MANUFACTURED BY SUMITOMO SEIKA CHEMICALS CO.,LTD. |
| D10 | RESIN PARTICLE | "FLOW BEAD PR" (POLYPROPYLENE PARTICLE (MELTING POINT 150°C, AVERAGE PARTICLE DIAMETER 10 µm)) MANUFACTURED BY SUMITOMO SEIKA CHEMICALS CO.,LTD. |
| D11 | AGGREGATE | "SYLOSPHERE C-1510" (SILICA PARTICLE, AVERAGE PARTICLE DIAMETER 10 µm) MANUFACTURED BY FUJI SILYSIA CHEMICAL LTD. |
| D12 | CURING CATALYST | "NACURE DDBSA SERIES 5225" (SODIUM DODECYLBENZENESULFONATE) MANUFACTURED BY KUSUMOTO CHEMICALS, LTD. |
| D13 | RESIN PARTICLE | "MBX-50" (ACRYLIC RESIN PARTICLE, AVERAGE PARTICLE DIAMETER 50 µm) MANUFACTURED BY SEKISUI PLASTICS CO., LTD. |
| D14 | RESIN PARTICLE | "MBX-100" (ACRYLIC RESIN PARTICLE, AVERAGE PARTICLE DIAMETER 100 µm) MANUFACTURED BY SEKISUI PLASTICS CO., LTD. |

**[Table 4-1]**

| No | METAL SHEET | PAINT BASE | RUST PREVENTIVE PAINT FILM | | | | | | | | | | | REMARKS |
|---|---|---|---|---|---|---|---|---|---|---|---|---|---|---|
| | | | CLEAR PAINT TYPE | FILM THICKNES S (µm) | RUST PREVENTIVE PIGMENT | | | | | | | | | |
| | | | | | RUST PREVENTIVE PIGMENT 1 | | RUST PREVENTIVE PIGMENT 2 | | RUST PREVENTIVE PIGMENT 3 | | RUST PREVENTIVE PIGMENT 4 | | TOTAL COVERAGE **RATIO** (%) | |
| | | | | | TYPE | COVERAGE RATIO (%) | TYPE | COVERAGE RATIO (%) | TYPE | COVERAGE RATIO (%) | TYPE | COVERAGE RATIO (%) | | |
| 1 | A1 | PRESENT | B1 | 10 | C1 | 20 | C2 | 20 | C5 | 5 | | | 45 | EXAMPLE |
| 2 | A1 | PRESENT | B1 | 10 | C1 | 20 | C2 | 20 | C5 | 5 | | | 45 | COMPARATIVE EXAMPLE |
| 3 | A1 | PRESENT | B1 | 10 | C1 | 20 | C2 | 20 | C5 | 5 | | | 45 | COMPARATIVE EXAMPLE |
| 4 | A1 | PRESENT | B1 | 10 | C1 | 20 | C2 | 20 | C5 | 5 | | | 45 | EXAMPLE |
| 5 | A1 | PRESENT | B1 | 10 | C1 | 20 | C2 | 20 | C5 | 5 | | | 45 | EXAMPLE |
| 6 | A1 | PRESENT | B1 | 10 | C1 | 20 | C2 | 20 | C5 | 5 | | | 45 | EXAMPLE |
| 7 | A1 | PRESENT | B1 | 10 | C1 | 20 | C2 | 20 | C5 | 5 | | | 45 | EXAMPLE |
| 8 | A1 | PRESENT | B1 | 10 | C1 | 20 | C2 | 20 | C5 | 5 | | | 45 | EXAMPLE |
| 9 | A1 | PRESENT | B1 | 10 | C1 | 20 | C2 | 20 | C5 | 5 | | | 45 | EXAMPLE |
| 10 | A1 | PRESENT | B1 | 10 | C1 | 20 | C2 | 20 | C5 | 5 | | | 45 | COMPARATIVE EXAMPLE |
| 11 | A1 | PRESENT | B1 | 10 | C1 | 20 | C2 | 20 | C5 | 5 | | | 45 | COMPARATIVE EXAMPLE |
| 12 | A1 | PRESENT | B1 | 10 | C1 | 20 | C2 | 20 | C5 | 5 | | | 45 | COMPARATIVE EXAMPLE |
| 13 | A1 | PRESENT | B1 | 10 | C1 | 20 | C2 | 20 | C5 | 5 | | | 45 | COMPARATIVE EXAMPLE |
| 14 | A1 | PRESENT | B1 | 10 | C1 | 20 | C2 | 20 | C5 | 5 | | | 45 | EXAMPLE |
| 15 | A1 | PRESENT | B1 | 10 | C1 | 20 | C2 | 20 | C5 | 5 | | | 45 | EXAMPLE |
| 16 | A1 | PRESENT | B1 | 10 | C1 | 20 | C2 | 20 | C5 | 5 | | | 45 | COMPARATIVE EXAMPLE |
| 17 | A1 | PRESENT | B1 | 10 | C1 | 20 | C2 | 20 | C5 | 5 | | | 45 | EXAMPLE |
| 18 | A1 | PRESENT | B1 | 10 | C1 | 20 | C2 | 20 | C5 | 5 | | | 45 | COMPARATIVE EXAMPLE |
| 19 | A1 | PRESENT | B1 | 10 | C1 | 20 | C2 | 20 | C5 | 5 | | | 45 | COMPARATIVE EXAMPLE |
| 20 | A1 | PRESENT | B1 | 10 | C1 | 20 | C2 | 20 | C5 | 5 | | | 45 | COMPARATIVE EXAMPLE |
| 21 | A1 | PRESENT | B1 | 10 | C1 | 20 | C2 | 20 | C5 | 5 | | | 45 | EXAMPLE |
| 22 | A1 | PRESENT | B1 | 10 | C1 | 20 | C2 | 20 | C5 | 5 | | | 45 | EXAMPLE |
| 23 | A1 | PRESENT | B1 | 10 | C1 | 20 | C2 | 20 | C5 | 5 | | | 45 | EXAMPLE |
| 24 | A1 | PRESENT | B1 | 10 | C1 | 20 | C2 | 20 | C5 | 5 | | | 45 | COMPARATIVE EXAMPLE |
| 25 | A1 | PRESENT | B1 | 10 | C1 | 20 | C2 | 20 | C5 | 5 | | | 45 | COMPARATIVE EXAMPLE |
| 26 | A1 | PRESENT | B1 | 10 | C1 | 20 | C2 | 20 | C5 | 5 | | | 45 | COMPARATIVE EXAMPLE |
| 27 | A1 | PRESENT | B1 | 10 | C1 | 20 | C2 | 20 | C5 | 5 | | | 45 | COMPARATIVE EXAMPLE |
| 28 | A1 | PRESENT | B1 | 10 | C1 | 20 | C2 | 20 | C5 | 5 | | | 45 | EXAMPLE |
| 29 | A1 | PRESENT | B1 | 10 | C1 | 20 | C2 | 20 | C5 | 5 | | | 45 | EXAMPLE |
| 30 | A1 | PRESENT | B1 | 10 | C1 | 20 | C2 | 20 | C5 | 5 | | | 45 | COMPARATIVE EXAMPLE |
| 31 | A1 | PRESENT | B1 | 10 | C1 | 20 | C2 | 20 | C5 | 5 | | | 45 | EXAMPLE |
| 32 | A1 | PRESENT | B1 | 10 | C1 | 20 | C2 | 20 | C5 | 5 | | | 45 | EXAMPLE |
| 33 | A1 | PRESENT | B1 | 10 | C1 | 20 | C2 | 20 | C5 | 5 | | | 45 | COMPARATIVE EXAMPLE |
| 34 | A1 | PRESENT | B1 | 10 | C1 | 20 | C2 | 20 | C5 | 5 | | | 45 | COMPARATIVE EXAMPLE |
| 35 | A1 | PRESENT | B1 | 10 | C1 | 20 | C2 | 20 | C5 | 5 | | | 45 | COMPARATIVE EXAMPLE |
| 36 | A1 | PRESENT | B1 | 10 | C1 | 20 | C2 | 20 | C5 | 5 | | | 45 | COMPARATIVE EXAMPLE |
| 37 | A1 | PRESENT | B1 | 10 | C1 | 20 | C2 | 20 | C5 | 5 | | | 45 | COMPARATIVE EXAMPLE |
| 38 | A1 | PRESENT | B1 | 10 | C1 | 20 | C2 | 20 | C5 | 5 | | | 45 | COMPARATIVE EXAMPLE |

**[Table 4-2]**

| No | METAL SHEET | PAINT BASE | RUST PREVENTIVE PAINT FILM | | | | | | | | | | | REMARKS |
|---|---|---|---|---|---|---|---|---|---|---|---|---|---|---|
| | | | CLEAR PAINT TYPE | FILM THICKNE SS (µm) | RUST PREVENTIVE PIGMENT | | | | | | | | | |
| | | | | | RUST PREVENTIVE PIGMENT 1 | | RUST PREVENTIVE PIGMENT 2 | | RUST PREVENTIVE PIGMENT 3 | | RUST PREVENTIVE PIGMENT 4 | | TOTAL COVERAGE RATIO (%) | |
| | | | | | TYPE | COVERAGE RATIO (%) | TYPE | COVERAGE RATIO (%) | TYPE | COVERAGE RATIO (%) | TYPE | COVERAGE RATIO (%) | | |
| 39 | A1 | PRESENT | B1 | 10 | C1 | 20 | C2 | 20 | C5 | 5 | | | 45 | EXAMPLE |
| 40 | A1 | PRESENT | B1 | 1 | C1 | 20 | C2 | 20 | C5 | 5 | | | 45 | COMPARATIVE EXAMPLE |
| 41 | A1 | PRESENT | B1 | 2 | C1 | 20 | C2 | 20 | C5 | 5 | | | 45 | COMPARATIVE EXAMPLE |
| 42 | A1 | PRESENT | B1 | 5 | C1 | 20 | C2 | 20 | C5 | 5 | | | 45 | EXAMPLE |
| 43 | A1 | PRESENT | B1 | 7 | C1 | 20 | C2 | 20 | C5 | 5 | | | 45 | EXAMPLE |
| 44 | A1 | PRESENT | B1 | 10 | C1 | 20 | C2 | 20 | C5 | 5 | | | 45 | EXAMPLE |
| 45 | A1 | PRESENT | B1 | 12 | C1 | 20 | C2 | 20 | C5 | 5 | | | 45 | EXAMPLE |
| 46 | A1 | PRESENT | B1 | 15 | C1 | 20 | C2 | 20 | C5 | 5 | | | 45 | EXAMPLE |
| 47 | A1 | PRESENT | B1 | 20 | C1 | 20 | C2 | 20 | C5 | 5 | | | 45 | COMPARATIVE EXAMPLE |
| 48 | A1 | PRESENT | B1 | 10 | C1 | 4 | C2 | 3 | C5 | 3 | | | 10 | COMPARATIVE EXAMPLE |
| 49 | A1 | PRESENT | B1 | 10 | C1 | 7 | C2 | 7 | C5 | 6 | | | 20 | COMPARATIVE EXAMPLE |
| 50 | A1 | PRESENT | B1 | 10 | C1 | 10 | C2 | 10 | C5 | 10 | | | 30 | EXAMPLE |
| 51 | A1 | PRESENT | B1 | 10 | C1 | 14 | C2 | 14 | C5 | 14 | | | 42 | EXAMPLE |
| 52 | A1 | PRESENT | B1 | 10 | C1 | 15 | C2 | 15 | C5 | 15 | | | 45 | EXAMPLE |
| 53 | A1 | PRESENT | B1 | 10 | C1 | 17 | C2 | 17 | C5 | 17 | | | 51 | EXAMPLE |
| 54 | A1 | PRESENT | B1 | 10 | C1 | 20 | C2 | 20 | C5 | 20 | | | 60 | EXAMPLE |
| 55 | A1 | PRESENT | B1 | 10 | C1 | 25 | C2 | 25 | C5 | 25 | | | 75 | COMPARATIVE EXAMPLE |
| 56 | A1 | PRESENT | B1 | 10 | C1 | 20 | C2 | 15 | C5 | 10 | | | 45 | EXAMPLE |
| 57 | A1 | PRESENT | B1 | 10 | C1 | 15 | C2 | 20 | C5 | 10 | | | 45 | EXAMPLE |
| 58 | A1 | PRESENT | B1 | 10 | C1 | 15 | C3 | 15 | C4 | 10 | C5 | 5 | 45 | EXAMPLE |
| 59 | A1 | PRESENT | B1 | 10 | C1 | 50 | | | | | | | 50 | EXAMPLE |
| 60 | A1 | PRESENT | B1 | 10 | C2 | 50 | | | | | | | 50 | EXAMPLE |
| 61 | A1 | PRESENT | B1 | 10 | C3 | 50 | | | | | | | 50 | EXAMPLE |
| 62 | A1 | PRESENT | B1 | 10 | C4 | 50 | | | | | | | 50 | EXAMPLE |
| 63 | A1 | PRESENT | B1 | 10 | C5 | 50 | | | | | | | 50 | EXAMPLE |
| 64 | A1 | ABSENT | B1 | 10 | C1 | 20 | C2 | 20 | C5 | 5 | | | 45 | EXAMPLE |
| 65 | A2 | PRESENT | B1 | 10 | C1 | 20 | C2 | 20 | C5 | 5 | | | 45 | EXAMPLE |
| 66 | A3 | PRESENT | B1 | 10 | C1 | 20 | C2 | 20 | C5 | 5 | | | 45 | EXAMPLE |
| 67 | A4 | PRESENT | B1 | 10 | C1 | 20 | C2 | 20 | C5 | 5 | | | 45 | EXAMPLE |
| 68 | A | PRESENT | B1 | 10 | C1 | 20 | C2 | 20 | C5 | 5 | | | 45 | COMPARATIVE EXAMPLE |
| 69 | A1 | PRESENT | B1 | 10 | C1 | 20 | C2 | 20 | C5 | 5 | | | 45 | EXAMPLE |
| 70 | A1 | PRESENT | B1 | 10 | C1 | 20 | C2 | 20 | C5 | 5 | | | 45 | EXAMPLE |
| 71 | A1 | PRESENT | B1 | 10 | C1 | 20 | C2 | 20 | C5 | 5 | | | 45 | EXAMPLE |
| 72 | A1 | PRESENT | B2 | 10 | C1 | 20 | C2 | 20 | C5 | 5 | | | 45 | EXAMPLE |
| 73 | A1 | PRESENT | B3 | 10 | C1 | 20 | C2 | 20 | C5 | 5 | | | 45 | EXAMPLE |
| 74 | A1 | PRESENT | B1 | 10 | C1 | 20 | C2 | 20 | C5 | 5 | | | 45 | EXAMPLE |
| 75 | A1 | PRESENT | B1 | 10 | C1 | 20 | C2 | 20 | C5 | 5 | | | 45 | EXAMPLE |

**[Table 4-3]**

| No | METAL SHEET | PAINT BASE | RUST PREVENTIVE PAINT FILM | | | | | | | | | | | REMARKS |
|---|---|---|---|---|---|---|---|---|---|---|---|---|---|---|
| | | | CLEAR PAINT TYPE | FILM THICKNE SS (µm) | RUST PREVENTIVE PIGMENT | | | | | | | | | |
| | | | | | RUST PREVENTIVE PIGMENT 1 | | RUST PREVENTIVE PIGMENT 2 | | RUST PREVENTIVE PIGMENT 3 | | RUST PREVENTIVE PIGMENT 4 | | TOTAL COVERAGE RATIO (%) | |
| | | | | | TYPE | COVERAGE RATIO (%) | TYPE | COVERAGE RATIO (%) | TYPE | COVERAGE RATIO (%) | TYPE | COVERAGE **RATIO** (%) | | |
| 76 | A1 | PRESENT | B1 | 10 | C1 | 20 | C2 | 20 | C5 | 5 | | | 45 | EXAMPLE |
| 77 | A1 | PRESENT | B1 | 10 | C1 | 20 | C2 | 20 | C5 | 5 | | | 45 | EXAMPLE |
| 78 | A1 | PRESENT | B1 | 10 | C1 | 20 | C2 | 20 | C5 | 5 | | | 45 | EXAMPLE |
| 79 | A1 | PRESENT | B1 | 10 | C1 | 20 | C2 | 20 | C5 | 5 | | | 45 | EXAMPLE |
| 80 | A1 | PRESENT | B1 | 10 | C1 | 20 | C2 | 20 | C5 | 5 | | | 45 | EXAMPLE |
| 81 | A1 | PRESENT | B1 | 10 | C1 | 20 | C2 | 20 | C5 | 5 | | | 45 | EXAMPLE |
| 82 | A1 | PRESENT | B1 | 10 | C1 | 20 | C2 | 20 | C5 | 5 | | | 45 | EXAMPLE |
| 83 | A1 | PRESENT | B1 | 10 | C1 | 20 | C2 | 20 | C5 | 5 | | | 45 | EXAMPLE |
| 84 | A1 | PRESENT | B1 | 10 | C1 | 20 | C2 | 20 | C5 | 5 | | | 45 | EXAMPLE |
| 85 | A1 | PRESENT | B1 | 10 | C1 | 20 | C2 | 20 | C5 | 5 | | | 45 | EXAMPLE |
| 86 | A1 | PRESENT | B1 | 10 | C1 | 20 | C2 | 20 | C5 | 5 | | | 45 | EXAMPLE |
| 87 | A4 | PRESENT | B1 | 10 | C1 | 20 | C2 | 20 | C5 | 5 | | | 45 | EXAMPLE |
| 88 | A4 | PRESENT | B1 | 10 | C1 | 20 | C2 | 20 | C5 | 5 | | | 45 | EXAMPLE |
| 89 | A4 | PRESENT | B1 | 10 | C1 | 20 | C2 | 20 | C5 | 5 | | | 45 | EXAMPLE |
| 90 | A4 | PRESENT | B1 | 10 | C1 | 20 | C2 | 20 | C5 | 5 | | | 45 | EXAMPLE |
| 91 | A4 | PRESENT | **B1** | 10 | C1 | 20 | C2 | 20 | C5 | 5 | | | 45 | EXAMPLE |
| 92 | A1 | PRESENT | B1 | 10 | C1 | 20 | C2 | 20 | C5 | 5 | | | 45 | EXAMPLE |
| 92 | A1 | PRESENT | B1 | 10 | C1 | 20 | C2 | 20 | C5 | 5 | | | 45 | EXAMPLE |
| 92 | A1 | PRESENT | B1 | 10 | C1 | 20 | C2 | 20 | C5 | 5 | | | 45 | EXAMPLE |

**[Table 5-1]**

| No | | | | | | | | | | | | | | REAR SURFACE COATING | | REMARKS |
|---|---|---|---|---|---|---|---|---|---|---|---|---|---|---|---|---|
| | PAINTING METHOD | FILM THICKNESS (µm) | HEATING TIME (s) | RESIN PARTICLE | | | | | AGGREGATE OR CURING CATALYST | | PARTICLE DIAMETER / FILM THICKNESS | MAXIMUM FILM THICKNESS / MINIMUM FILM THICKNESS | RESIN PARTICLE COVERAGE | RUST PREVENTIVE PAINT FILM | OUTERMOST LAYER PAINT FILM | |
| | | | | RESIN PARTICLE 1 | | RESIN PARTICLE 2 | | TOTAL COVERAGE RATIO (%) | TYPE | COVERAGE RATIO (%) | | | | | | |
| | | | | TYPE | COVERAGE RATIO (%) | TYPE | COVERAGE RATIO (%) | | | | | | | | | |
| 1 | CURTAIN | 10 | 12 | D6 | 15 | | | 15 | | | 3.2 | | ○ | | | EXAMPLE |
| 2 | CURTAIN | 10 | 12 | | | | | Q | | | 0.0 | | ○ | | | COMPARATIVE EXAMPLE |
| 3 | CURTAIN | 10 | 12 | D6 | 1 | | | 1 | | | 18 | | ○ | | | COMPARATIVE EXAMPLE |
| 4 | CURTAIN | 10 | 12 | D6 | 2 | | | 2 | | | 2.4 | | ○ | | | EXAMPLE |
| 5 | CURTAIN | 10 | 12 | D6 | 5 | | | 5 | | | 3.0 | | ○ | | | EXAMPLE |
| 6 | CURTAIN | 10 | 12 | D6 | 10 | | | 10 | | | 3.0 | | ○ | | | EXAMPLE |
| 7 | CURTAIN | 10 | 12 | D6 | 20 | | | 20 | | | 3.2 | | ○ | | | EXAMPLE |
| 8 | CURTAIN | 10 | 12 | D6 | 30 | | | 30 | | | 3.3 | | ○ | | | EXAMPLE |
| 9 | CURTAIN | 10 | 12 | D6 | 35 | | | 35 | | | 3.2 | | ○ | | | EXAMPLE |
| 10 | CURTAIN | 10 | 12 | D1 | 15 | | | 15 | | | 0.2 | | ○ | | | COMPARATIVE EXAMPLE |
| 11 | CURTAIN | 10 | 12 | D2 | 15 | | | 15 | | | 0.4 | | ○ | | | COMPARATIVE EXAMPLE |
| 12 | CURTAIN | 10 | 12 | D3 | 15 | | | 15 | | | 0.5 | | ○ | | | COMPARATIVE EXAMPLE |
| 13 | CURTAIN | 10 | 12 | D4 | 15 | | | 15 | | | 1.1 | | ○ | | | COMPARATIVE EXAMPLE |
| 14 | CURTAIN | 10 | 12 | D5 | 15 | | | 15 | | | 2.1 | | ○ | | | EXAMPLE |
| 15 | CURTAIN | 10 | 12 | D6 | 10 | D3 | 5 | 15 | | | 3.1 | | ○ | | | EXAMPLE |
| 16 | BAR | | 12 | D6 | 15 | | | 15 | | | 1.8 | | × | | | COMPARATIVE EXAMPLE |
| 17 | CURTAIN | 10 | 12 | D8 | 15 | | | 15 | | | 2.1 | | ○ | | | EXAMPLE |
| 18 | CURTAIN | 5 | 12 | D1 | 15 | | | 15 | | | 0.5 | | ○ | | | COMPARATIVE EXAMPLE |
| 19 | CURTAIN | 5 | 12 | D2 | 15 | | | 15 | | | 0.8 | | ○ | | | COMPARATIVE EXAMPLE |
| 20 | CURTAIN | 5 | 12 | D3 | 15 | | | 15 | | | 1.2 | | ○ | | | COMPARATIVE EXAMPLE |
| 21 | CURTAIN | 5 | 12 | D4 | 15 | | | 15 | | | 2.3 | | ○ | | | EXAMPLE |
| 22 | CURTAIN | 5 | 12 | D5 | 15 | | | 15 | | | 4.0 | | ○ | | | EXAMPLE |
| 23 | CURTAIN | 5 | 12 | D6 | 10 | D3 | 5 | 15 | | | 6.0 | | ○ | | | EXAMPLE |
| 24 | CURTAIN | 10 5 | 12 | D7 | 15 | | | 15 | | | 1.5 | | ○ | | | COMPARATIVE EXAMPLE |
| 25 | CURTAIN | 5 | 12 | D9 | 15 | | | 15 | | | 1.4 | | × | | | COMPARATIVE EXAMPLE |
| 26 | CURTAIN | 5 | 12 | D10 | 15 | | | 15 | | | 1.8 | | × | | | COMPARATIVE EXAMPLE |
| 27 | CURTAIN | 5 | 12 | | | | | 0 | D11 | 3 | 1.4 | | ○ | | | COMPARATIVE EXAMPLE |
| 28 | CURTAIN | 5 | 12 | | | | | 0 | D11 | 15 | 2.3 | | ○ | | | EXAMPLE |
| 29 | CURTAIN | 5 | 12 | | | | | 0 | D11 | 20 | 2.3 | | ○ | | | EXAMPLE |
| 30 | CURTAIN | 5 | 12 | | | | | 0 | D12 | 0.5 | | | | | | COMPARATIVE EXAMPLE |
| 31 | CURTAIN | 5 | 12 | | | | | 0 | D12 | 2 | | | | | | EXAMPLE |
| 32 | CURTAIN | 5 | 12 | | | | | 0 | D12 | 4 | | | | | | EXAMPLE |
| 33 | BAR | 5 | 12 | D4 | 15 | | | 15 | | | 1.9 | | × | | | COMPARATIVE EXAMPLE |
| 34 | CURTAIN | 15 | 12 | D1 | 15 | | | 15 | | | 0.1 | | ○ | | | COMPARATIVE EXAMPLE |
| 35 | CURTAIN | 15 | 12 | D2 | 15 | | | 15 | | | 0.3 | | ○ | | | COMPARATIVE EXAMPLE |
| 36 | CURTAIN | 15 | 12 | D3 | 15 | | | 15 | | | 0.4 | | ○ | | | COMPARATIVE EXAMPLE |
| 37 | CURTAIN | 15 | 12 | D4 | 15 | | | 15 | | | 0.8 | | ○ | | | COMPARATIVE EXAMPLE |
| 38 | CURTAIN | 15 | 12 | D5 | 15 | | | 15 | | | 1.3 | | ○ | | | COMPARATIVE EXAMPLE |

**[Table 5-2]**

| No | | | | | | | | | | | | | | REAR SURFACE COATING | | REMARKS |
|---|---|---|---|---|---|---|---|---|---|---|---|---|---|---|---|---|
| | PAINTING METHOD | FILM THICKNESS (µm) | HEATING TIME (s) | RESIN PARTICLE | | | | | AGGREGATE OR CURING CATALYST | | PARTICLE DIAMETER / FILM THICKNESS | MAXIMUM FILM THICKNESS / MINIMUM FILM THICKNESS | RESIN PARTICLE COVERAGE | RUST PREVENTIVE PAINT FILM | OUTERMOST LAYER PAINT FILM | |
| | | | | RESIN PARTICLE 1 | | RESIN PARTICLE 2 | | TOTAL COVERAGE RATIO (%) | TYPE | COVERAGE RATIO (%) | | | | | | |
| | | | | TYPE | COVERAGE RATIO (%) | TYPE | COVERAGE RATIO (%) | | | | | | | | | |
| 39 | CURTAIN | 15 | 12 | D6 | 10 | D3 | 5 | 15 | | | 2.1 | | ○ | | | EXAMPLE |
| 40 | CURTAIN | 10 | 12 | D6 | 15 | | | 15 | | | 3.2 | | ○ | | | COMPARATIVE EXAMPLE |
| 41 | CURTAIN | 10 | 12 | D6 | 15 | | | 15 | | | 3.2 | | ○ | | | COMPARATIVE EXAMPLE |
| 42 | CURTAIN | 10 | 12 | D6 | 15 | | | 15 | | | 3.2 | | ○ | | | EXAMPLE |
| 43 | CURTAIN | 10 | 12 | D6 | 15 | | | 15 | | | 3.2 | | ○ | | | EXAMPLE |
| 44 | CURTAIN | 10 | 12 | D6 | 15 | | | 15 | | | 3.2 | | ○ | | | EXAMPLE |
| 45 | CURTAIN | 10 | 12 | D6 | 15 | | | 15 | | | 3.2 | | ○ | | | EXAMPLE |
| 46 | CURTAIN | 10 | 12 | D6 | 15 | | | 15 | | | 3.2 | | ○ | | | EXAMPLE |
| 47 | CURTAIN | 10 | 12 | D6 | 15 | | | 15 | | | 3.2 | | ○ | | | COMPARATIVE EXAMPLE |
| 48 | CURTAIN | 10 | 12 | D6 | 15 | | | 15 | | | 3.2 | | ○ | | | COMPARATIVE EXAMPLE |
| 49 | CURTAIN | 10 | 12 | D6 | 15 | | | 15 | | | 3.2 | | ○ | | | COMPARATIVE EXAMPLE |
| 50 | CURTAIN | 10 | 12 | D6 | 15 | | | 15 | | | 3.2 | | ○ | | | EXAMPLE |
| 51 | CURTAIN | 10 | 12 | D6 | 15 | | | 15 | | | 3.2 | | ○ | | | EXAMPLE |
| 52 | CURTAIN | 10 | 12 | D6 | 15 | | | 15 | | | 3.2 | | ○ | | | EXAMPLE |
| 53 | CURTAIN | 10 | 12 | D6 | 15 | | | 15 | | | 3.2 | | ○ | | | EXAMPLE |
| 54 | CURTAIN | 10 | 12 | D6 | 15 | | | 15 | | | 3.2 | | ○ | | | EXAMPLE |
| 55 | CURTAIN | 10 | 12 | D6 | 15 | | | 15 | | | 3.2 | | ○ | | | COMPARATIVE EXAMPLE |
| 56 | CURTAIN | 10 | 12 | D6 | 15 | | | 15 | | | 3.2 | | ○ | | | EXAMPLE |
| 57 | CURTAIN | 10 | 12 | D6 | 15 | | | 15 | | | 3.2 | | ○ | | | EXAMPLE |
| 58 | CURTAIN | 10 | 12 | D6 | 15 | | | 15 | | | 3.2 | | ○ | | | EXAMPLE |
| 59 | CURTAIN | 10 | 12 | D6 | 15 | | | 15 | | | 3.2 | | ○ | | | EXAMPLE |
| 60 | CURTAIN | 10 | 12 | D6 | 15 | | | 15 | | | 3.2 | | ○ | | | EXAMPLE |
| 61 | CURTAIN | 10 | 12 | D6 | 15 | | | 15 | | | 3.2 | | ○ | | | EXAMPLE |
| 62 | CURTAIN | 10 | 12 | D6 | 15 | | | 15 | | | 3.2 | | ○ | | | EXAMPLE |
| 63 | CURTAIN | 10 | 12 | D6 | 15 | | | 15 | | | 3.2 | | ○ | | | EXAMPLE |
| 64 | CURTAIN | 10 | 12 | D6 | 15 | | | 15 | | | 3.2 | | ○ | | | EXAMPLE |
| 65 | CURTAIN | 10 | 12 | D6 | 15 | | | 15 | | | 3.2 | | ○ | | | EXAMPLE |
| 66 | CURTAIN | 10 | 12 | D6 | 15 | | | 15 | | | 3.2 | | ○ | | | EXAMPLE |
| 67 | CURTAIN | 10 | 12 | D6 | 15 | | | 15 | | | 3.2 | | ○ | | | EXAMPLE |
| 68 | CURTAIN | 10 | 12 | D6 | 15 | | | 15 | | | 3.2 | | ○ | | | COMPARATIVE EXAMPLE |
| 69 | CURTAIN | 10 | 12 | D6 | 15 | | | 15 | | | 3.2 | | ○ | SAME AS NO 1 | SAME AS NO 1 | EXAMPLE |
| 70 | CURTAIN | 10 | 12 | D6 | 15 | | | 15 | | | 3.2 | | ○ | SAME AS NO 2 | SAME AS NO 1 | EXAMPLE |
| 71 | CURTAIN | 10 | 12 | D6 | 15 | | | 15 | | | 3.2 | | ○ | NO COATING | NO COATING | EXAMPLE |
| 72 | CURTAIN | 10 | 12 | D6 | 15 | | | 15 | | | 3.2 | | ○ | | | EXAMPLE |
| 73 | CURTAIN | 10 | 12 | D6 | 15 | | | 15 | | | 3.2 | | ○ | | | EXAMPLE |
| 74 | CURTAIN | 10 | 24 | D8 | 15 | | | 15 | | | 2.1 | | ○ | | | EXAMPLE |
| 75 | CURTAIN | 10 | 48 | D8 | 15 | | | 15 | | | 2.1 | | × | | | EXAMPLE |

**[Table 5-3]**

| No | | | | | | | | | | | | | | REAR SURFACE COATING | | REMARKS |
|---|---|---|---|---|---|---|---|---|---|---|---|---|---|---|---|---|
| | PAINTING METHOD | FILM THICKNESS (µm) | HEATING TIME (s) | RESIN PARTICLE | | | | | AGGREGATE OR CURING CATALYST | | PARTICLE DIAMETER / FILM THICKNESS | Maximum FILM THICKNESS / MINIMUM FILM THICKNESS | RESIN PARTICLE COVERAGE | RUST PREVENTIVE PAINT FILM | OUTERMOST LAYER PAINT FILM | |
| | | | | RESIN PARTICLE 1 | | RESIN PARTICLE 2 | | TOTAL COVERAGE RATIO (%) | TYPE | COVERAGE RATIO (%) | | | | | | |
| | | | | TYPE | COVERAGE RATIO (%) | TYPE | COVERAGE RATIO (%) | | | | | | | | | |
| 76 | CURTAIN | 12 | 12 | D6 | 5 | | | 5 | | | 2.5 | 4 | ○ | | | EXAMPLE |
| 77 | CURTAIN | 8 | 12 | D6 | 15 | | | 15 | | | 3.8 | 8 | O | | | EXAMPLE |
| 78 | CURTAIN | 12 | 12 | D6 | 15 | | | 15 | | | 2.5 | 5 | ○ | | | EXAMPLE |
| 79 | CURTAIN | 8 | 12 | D6 | 20 | | | 20 | | | 3.8 | 10 | O | | | EXAMPLE |
| 80 | CURTAIN | 12 | 12 | D6 | 20 | | | 20 | | | 2.5 | 7 | ○ | | | EXAMPLE |
| 81 | CURTAIN | 20 | 12 | D13 | 15 | | | 15 | | | 2.5 | 6 | O | | | EXAMPLE |
| 82 | CURTAIN | 20 | 12 | D13 | 15 | | | 20 | | | 2.5 | 9 | ○ | | | EXAMPLE |
| 83 | CURTAIN | 20 | 12 | D13 | 15 | | | 25 | | | 2.5 | 12 | O | | | EXAMPLE |
| 84 | CURTAIN | 15 | 12 | D13 | 15 | | | 20 | | | 3.3 | 17 | ○ | | | EXAMPLE |
| 85 | CURTAIN | 13 | 12 | D13 | 15 | | | 20 | | | 3.8 | 21 | ○ | | | EXAMPLE |
| 86 | CURTAIN | 25 | 12 | D14 | 15 | | | 20 | | | 4.0 | 23 | ○ | | | EXAMPLE |
| 87 | CURTAIN | 20 | 12 | D13 | 15 | | | 15 | | | 2.5 | 6 | O | | | EXAMPLE |
| 88 | CURTAIN | 20 | 12 | D13 | 15 | | | 20 | | | 2.5 | 9 | ○ | | | EXAMPLE |
| 89 | CURTAIN | 20 | 12 | D13 | 15 | | | 25 | | | 2.5 | 12 | ○ | | | EXAMPLE |
| 90 | CURTAIN | 15 | 12 | D13 | 15 | | | 20 | | | 3.3 | 17 | ○ | | | EXAMPLE |
| 91 | CURTAIN | 13 | 12 | D13 | 15 | | | 20 | | | 3.8 | 21 | ○ | | | EXAMPLE |
| 92 | CURTAIN | 20 | 12 | D1 | 50 | | | 50 | | | 0.1 | 1.2 | ○ | | | EXAMPLE |
| 93 | CURTAIN | 20 | 12 | D2 | 50 | | | 50 | | | 0.2 | 1.3 | O | | | EXAMPLE |
| 94 | CURTAIN | 20 | 12 | D3 | 50 | | | 50 | | | 0.3 | 1.4 | ○ | | | EXAMPLE |

**[Table 6-1]**

| No | EVALUATION | | | | | | REMARKS |
|---|---|---|---|---|---|---|---|
| | GLOSSINESS | CORROSION RESISTANCE | | FLAW RESISTANCE | ROUGHNESS | PARTICLE FALL-OFF | |
| | | CORROSION RESISTANCE 1 | CORROSION RESISTANCE 2 | | | | |
| 1 | 10 | 4 | | 4 | | O | EXAMPLE |
| 2 | 60 | 4 | | 2 | × | | COMPARATIVE EXAMPLE |
| 3 | 40 | 4 | | 2 | | ○ | COMPARATIVE EXAMPLE |
| 4 | 19 | 4 | | 4 | | O | EXAMPLE |
| 5 | 18 | 4 | | 4 | | ○ | EXAMPLE |
| 6 | 15 | 4 | | 4 | | O | EXAMPLE |
| 7 | 8 | 4 | | 4 | | ○ | EXAMPLE |
| 8 | 7 | 4 | | 4 | | ○ | EXAMPLE |
| 9 | 5 | 4 | | 3 | | ○ | EXAMPLE |
| 10 | 60 | 5 | | 2 | | ○ | COMPARATIVE EXAMPLE |
| 11 | 55 | 5 | | 2 | | ○ | COMPARATIVE EXAMPLE |
| 12 | 53 | 5 | | 2 | | ○ | COMPARATIVE EXAMPLE |
| 13 | 45 | 4 | | 2 | | ○ | COMPARATIVE EXAMPLE |
| 14 | 20 | 4 | | 4 | | ○ | EXAMPLE |
| 15 | 10 | 4 | | 4 | | O | EXAMPLE |
| 16 | 40 | 2 | | 2 | | ○ | COMPARATIVE EXAMPLE |
| 17 | 18 | 5 | | 4 | | ○ | EXAMPLE |
| 18 | 45 | 4 | | 2 | | ○ | COMPARATIVE EXAMPLE |
| 19 | 40 | 3 | | 2 | | ○ | COMPARATIVE EXAMPLE |
| 20 | 38 | 3 | | 2 | | ○ | COMPARATIVE EXAMPLE |
| 21 | 15 | 3 | | 4 | | O | EXAMPLE |
| 22 | 6 | 3 | | 4 | | × | EXAMPLE |
| 23 | 5 | 3 | | 4 | | ○ | EXAMPLE |
| 24 | 30 | 3 | | 2 | | ○ | COMPARATIVE EXAMPLE |
| 25 | 35 | 3 | | 2 | | ○ | COMPARATIVE EXAMPLE |
| 26 | 25 | 3 | | 2 | | ○ | COMPARATIVE EXAMPLE |
| 27 | 40 | 3 | | 2 | × | | COMPARATIVE EXAMPLE |
| 28 | 16 | 3 | | 3 | ○ | | EXAMPLE |
| 29 | 13 | 3 | | 3 | ○ | | EXAMPLE |
| 30 | 50 | 3 | | 2 | × | | COMPARATIVE EXAMPLE |
| 31 | 10 | 3 | | 3 | ○ | | EXAMPLE |
| 32 | 9 | 3 | | 3 | ○ | | EXAMPLE |
| 33 | 25 | 2 | | 2 | | ○ | COMPARATIVE EXAMPLE |
| 34 | 60 | 5 | | 2 | | ○ | COMPARATIVE EXAMPLE |
| 35 | 60 | 5 | | 2 | | ○ | COMPARATIVE EXAMPLE |
| 36 | 56 | 5 | | 2 | | ○ | COMPARATIVE EXAMPLE |
| 37 | 50 | 5 | | 2 | | ○ | COMPARATIVE EXAMPLE |
| 38 | 38 | 5 | | 2 | | ○ | COMPARATIVE EXAMPLE |

**[Table 6-2]**

| No | EVALUATION | | | | | | REMARKS |
|---|---|---|---|---|---|---|---|
| | GLOSSINESS | CORROSION RESISTANCE | | FLAW RESISTANCE | ROUGHNES S | PARTICLE FALL-OFF | |
| | | CORROSION RESISTANCE 1 | CORROSION RESISTANCE 2 | | | | |
| 39 | 18 | 5 | | 4 | | ○ | EXAMPLE |
| 40 | 10 | 2 | | 4 | | ○ | COMPARATIVE EXAMPLE |
| 41 | 10 | 2 | | 4 | | ○ | COMPARATIVE EXAMPLE |
| 42 | 10 | 3 | | 4 | | ○ | EXAMPLE |
| 43 | 10 | 3 | | 4 | | ○ | EXAMPLE |
| 44 | 10 | 4 | | 4 | | ○ | EXAMPLE |
| 45 | 10 | 4 | | 4 | | ○ | EXAMPLE |
| 46 | 10 | 4 | | 4 | | ○ | EXAMPLE |
| 47 | 10 | 2 | | 4 | | ○ | COMPARATIVE EXAMPLE |
| 48 | 10 | 2 | | 4 | | ○ | COMPARATIVE EXAMPLE |
| 49 | 10 | 2 | | 4 | | ○ | COMPARATIVE EXAMPLE |
| 50 | 10 | 3 | | 4 | | ○ | EXAMPLE |
| 51 | 10 | 4 | | 4 | | ○ | EXAMPLE |
| 52 | 10 | 4 | | 4 | | ○ | EXAMPLE |
| 53 | 10 | 4 | | 3 | | ○ | EXAMPLE |
| 54 | 10 | 4 | | 3 | | ○ | EXAMPLE |
| 55 | 10 | 2 | | 2 | | ○ | COMPARATIVE EXAMPLE |
| 56 | 10 | 4 | | 4 | | ○ | EXAMPLE |
| 57 | 10 | 4 | | 4 | | ○ | EXAMPLE |
| 58 | 10 | 4 | | 4 | | ○ | EXAMPLE |
| 59 | 10 | 3 | | 4 | | ○ | EXAMPLE |
| 60 | 10 | 3 | | 4 | | ○ | EXAMPLE |
| 61 | 10 | 3 | | 4 | | ○ | EXAMPLE |
| 62 | 10 | 3 | | 4 | | ○ | EXAMPLE |
| 63 | 10 | 3 | | 4 | | ○ | EXAMPLE |
| 64 | 10 | 3 | | 4 | | ○ | EXAMPLE |
| 65 | 10 | 4 | | 4 | | ○ | EXAMPLE |
| 66 | 10 | 4 | | 4 | | ○ | EXAMPLE |
| 67 | 10 | 5 | | 4 | | ○ | EXAMPLE |
| 68 | 10 | 1 | | 4 | | ○ | COMPARATIVE EXAMPLE |
| 69 | 10 | 4 | 2 | 4 | | ○ | EXAMPLE |
| 70 | 10 | 4 | 1 | 4 | | ○ | EXAMPLE |
| 71 | 10 | 4 | 1 | 4 | | ○ | EXAMPLE |
| 72 | 9 | 4 | | 4 | | ○ | EXAMPLE |
| 73 | 8 | 4 | | 4 | | ○ | EXAMPLE |
| 74 | 18 | 4 | | 4 | | ○ | EXAMPLE |
| 75 | 18 | 3 | | 4 | | ○ | EXAMPLE |

**[Table 6-3]**

| No | EVALUATION | | | | | | REMARKS |
|---|---|---|---|---|---|---|---|
| | GLOSSINESS | CORROSION RESISTANCE | | FLAW RESISTANCE | ROUGHNESS | PARTICLE FALL-OFF | |
| | | CORROSION RESISTANCE 1 | CORROSION RESISTANCE 2 | | | | |
| 76 | 20 | 4 | | 4 | | ○ | EXAMPLE |
| 77 | 7 | 3 | | 4 | | ○ | EXAMPLE |
| 78 | 9 | 4 | | 4 | | ○ | EXAMPLE |
| 79 | 5 | 3 | | 4 | | ○ | EXAMPLE |
| 80 | 8 | 4 | | 4 | | ○ | EXAMPLE |
| 81 | 8 | 4 | | 4 | | ○ | EXAMPLE |
| 82 | 7 | 4 | | 4 | | ○ | EXAMPLE |
| 83 | 5 | 3 | | 4 | | ○ | EXAMPLE |
| 84 | 5 | 3 | | 4 | | ○ | EXAMPLE |
| 85 | 5 | 3 | | 3 | | × | EXAMPLE |
| 86 | 5 | 3 | | 3 | | × | EXAMPLE |
| 87 | 8 | 5 | | 4 | | ○ | EXAMPLE |
| 88 | 7 | 5 | | 4 | | ○ | EXAMPLE |
| 89 | 5 | 5 | | 4 | | ○ | EXAMPLE |
| 90 | 5 | 5 | | 4 | | ○ | EXAMPLE |
| 91 | 5 | 5 | | 3 | | × | EXAMPLE |
| 92 | 20 | 3 | | 3 | | × | EXAMPLE |
| 93 | 18 | 3 | | 3 | | × | EXAMPLE |
| 94 | 17 | 3 | | 3 | | × | EXAMPLE |

As is clear from Table 4-1 to Table 6-3 above, the sample materials corresponding to the examples of the present invention are shown to be capable of achieving both the matte appearance with excellent low glossiness and the high corrosion resistance. Further, the sample materials are shown to secondarily exhibit high flaw resistance. Further, the sample materials corresponding to the configurations satisfying the preferred aspect of the present invention are shown to exhibit the effect of suppressing the fall-off of the particles. On the other hand, the sample materials corresponding to the comparative examples of the present invention were unacceptable in at least either the low glossiness or the corrosion resistance.

No. 2 contained no resin particle in the outermost layer paint film layer, and No. 3 contained resin particles but was low in percentage thereof. Besides, No. 27 contained no resin particle in the outermost layer paint film layer, and contained the aggregate but was low in percentage thereof. Besides, No. 30 contained no resin particle in the outermost layer paint film layer, and contained the curing catalyst but was low in percentage thereof. Therefore, it is considered that the glossiness was outside of the range and the desired design could not be realized.

Nos. 10 to 13, 16, 18 to 20, 24 to 26, and 33 to 38 were less than twice the disclosure of this application in the ratio (particle diameter/film thickness) between the average particle diameter φ₁₀ and the average film thickness T. Therefore, it is considered that the glossiness was outside of the range and the desired design could not be realized.

Nos. 40 and 41 were less than 5 µm in the film thickness of the rust preventive paint film (see Table 4-1), and therefore it is considered that the effect of suppressing the corrosion against the corrosion factor possibly intruding through the interface between the thin film portion or the particle 101 and the binder resin 103 was not sufficient. Therefore, it is considered that the desired corrosion resistance could not be obtained. Besides, No. 47 was more than 15 µm in the film thickness of the rust preventive paint film, and therefore it is considered that the paint defect occurred. Therefore, it is considered that the desired corrosion resistance could not be obtained.

Nos. 48 and 49 were less than 30% in the coverage ratio of the rust preventive pigment (see Table 4-1), and therefore it is considered that the effect of suppressing the corrosion against the corrosion factor possibly intruding through the interface between the thin film portion or the particle 101 and the binder resin 103 was not sufficient. Therefore, it is considered that the desired corrosion resistance could not be obtained. Besides, No. 55 was more than 60% in the coverage ratio of the rust preventive pigment (see Table 4-1), and therefore it is considered that the adhesiveness between the rust preventive paint film layer 20 and the steel sheet 10, particularly, the adhesiveness at the worked portion was not sufficient. Therefore, it is considered that the desired corrosion resistance could not be obtained.

No. 68 was not provided with the plating layer on the surface of the steel sheet 10 (using the metal sheet A5), and therefore it is considered that the desired corrosion resistance could not be obtained.

Preferred embodiments of the present invention have been explained above in detail with reference to the attached drawings, but the present invention is not limited to the embodiments. It should be understood that various changes and modifications are readily apparent to those skilled in the art who have the common general knowledge in the technical field to which the present invention pertains, within the scope of the technical spirit as set forth in claims, and they should also be covered by the technical scope of the present invention.

The embodiments disclosed herein are examples in all respects and should not be considered to be restrictive. Various omissions, substitutions, and changes may be made in the embodiments without departing from the scope and the spirit of the attached claims and a later-explained technical scope of the present invention. For example, configuration requirements of the above embodiments can be arbitrarily combined within a range that does not impair the effects thereof. Further, from the arbitrary combination, the operations and effects about the configuration requirements relating to the combination can be naturally obtained, and other operations and other effects apparent to those skilled in the art are obtained from the description herein.

Besides, the effects explained herein are merely explanatory or illustrative in all respects and not restrictive. In other words, the technique relating to the present invention can offer other effects apparent to those skilled in the art from the description herein in addition to or in place of the above effects.

Note that the following configurations also belong to the technical scope of the present invention.
[1] A painted steel sheet including
   two or more paint film layers including a rust preventive paint film layer on at least one side of a steel sheet having a Zn-containing plating layer, wherein:
   a 60-degree specular glossiness Gs (60°) specified in JIS Z 8741:1997 of the paint film layer on at least one face of the steel sheet is 20% or less;
   an average film thickness of the rust preventive paint film layer is 5 µm or more and 15 µm or less;
   the rust preventive paint film layer contains a binder resin, a cross-linking agent, and a rust preventive pigment; and
   in a cross section obtained by cutting the paint film layer in a thickness direction at an arbitrary position, a coverage ratio of the rust preventive pigment to a total area of the rust preventive paint film layer is 30% or more and 60% or less in terms of area ratio.
[2] The painted steel sheet according to the above [1], wherein
   the rust preventive pigment contains at least one or more of Si, P, Mg, and V.
[3] The painted steel sheet according to the above [2], wherein
   the Si contains any one or more of calcium ion-exchanged silica and magnesium ion-exchanged silica, the P contains any one or more of zinc phosphate, magnesium dihydrogen phosphate, and aluminium dihydrogen triphosphate, and the Mg contains any one or more of magnesium dihydrogen phosphate, magnesium oxide, and magnesium hydroxide.
[4] The painted steel sheet according to any one of the above [1] to [3], wherein:
   on the face of the steel sheet where the 60-degree specular glossiness Gs (60°) is 20% or less, the two or more paint film layers have the rust preventive paint film layer at a lower layer and have a colored paint film layer at an outermost layer located on a farthest side from the steel sheet, and the colored paint film layer contains a resin particle, and a binder resin, a cross-linking agent, and a color pigment as a film-forming component; and
   in the cross section, an average particle diameter of the resin particle is two times or more and five times or less an average film thickness at a portion not having the resin particle of the outermost layer paint film layer.
   Where the average particle diameter is a value obtained by measuring, in one observation visual field region in the cross section, circle-equivalent diameters of the resin particles existing in the observation visual field region, calculating an average value of upper two circle-equivalent diameters in descending order of the circle-equivalent diameters, and further averaging the averaged values similarly obtained for the observation visual field regions at ten arbitrary locations, by a number of fields of view.
[5] The painted steel sheet according to the above [4], wherein
   the coverage ratio of the resin particles to a total area of the outermost layer paint film layer is 5% or more and 30% or less in terms of area ratio.
[6] The painted steel sheet according to the above [4] or [5], wherein
   in the cross section, a projecting portion of the resin particle projecting from a position on a surface at the portion not containing the resin particle of the outermost layer paint film layer is covered, at half or more of a length along an outer peripheral portion of the projecting portion, with the film-forming component having a thickness of 0.5 µm or more.
[7] The painted steel sheet according to any one of the above [4] to [6], wherein
   the resin particle is a resin particle made of an acrylic resin.
[8] The painted steel sheet according to any one of the above [4] to [7], wherein
   the binder resin is a binder resin made of an acrylic resin or a polyester resin.
[9] The painted steel sheet according to any one of the above [1] to [8] having a characteristic selected from any one or two of a surface roughness of the steel sheet being 2 µm or more in Ra on the face of the steel sheet where the 60-degree specular glossiness Gs (60°) is 20% or less, and the paint film layer containing 15% or more of an aggregate composed of a pigment containing silica.

### EXPLANATION OF CODES

- 1: painted steel sheet
- 10: steel sheet
- 20: rust preventive paint film layer
- 30: outermost paint film layer
- 101: particle
- 103: binder resin

## Claims

1. A painted steel sheet comprising
two or more paint film layers including a rust preventive paint film layer on at least one side of a steel sheet having a Zn-containing plating layer, wherein:
a 60-degree specular glossiness Gs (60°) specified in JIS Z 8741:1997 of the paint film layer on at least one face of the steel sheet is 20% or less;
an average film thickness of the rust preventive paint film layer is 5 µm or more and 15 µm or less;
the rust preventive paint film layer contains a binder resin, a cross-linking agent, and a rust preventive pigment; and
in a cross section obtained by cutting the paint film layer in a thickness direction at an arbitrary position, a coverage ratio of the rust preventive pigment to a total area of the rust preventive paint film layer is 30% or more and 60% or less in terms of area ratio.

2. The painted steel sheet according to claim 1, wherein
the rust preventive pigment contains at least one or more of Si, P, Mg, and V.

3. The painted steel sheet according to claim 2, wherein
the Si contains any one or more of calcium ion-exchanged silica and magnesium ion-exchanged silica, the P contains any one or more of zinc phosphate, magnesium dihydrogen phosphate, and aluminium dihydrogen triphosphate, and the Mg contains any one or more of magnesium dihydrogen phosphate, magnesium oxide, and magnesium hydroxide.

4. The painted steel sheet according to claim 1, wherein:
on the face of the steel sheet where the 60-degree specular glossiness Gs (60°) is 20% or less, the two or more paint film layers have the rust preventive paint film layer at a lower layer and have a colored paint film layer at an outermost layer located on a farthest side from the steel sheet, and the colored paint film layer contains a resin particle, and a binder resin, a cross-linking agent, and a color pigment as a film-forming component; and
in the cross section, an average particle diameter of the resin particle is two times or more and five times or less an average film thickness at a portion not having the resin particle of the colored paint film layer.
Where the average particle diameter is a value obtained by measuring, in one observation visual field region in the cross section, circle-equivalent diameters of the resin particles existing in the observation visual field region, calculating an average value of upper two circle-equivalent diameters in descending order of the circle-equivalent diameters, and further averaging the averaged values similarly obtained for the observation visual field regions at ten arbitrary locations, by a number of fields of view.

5. The painted steel sheet according to claim 4, wherein
the coverage ratio of the resin particles to a total area of the colored paint film layer is 5% or more and 30% or less in terms of area ratio.

6. The painted steel sheet according to claim 4, wherein
in the cross section, a projecting portion of the resin particle projecting from a position on a surface at the portion not containing the resin particle of the colored paint film layer is covered, at half or more of a length along an outer peripheral portion of the projecting portion, with the film-forming component having a thickness of 0.5 µm or more.

7. The painted steel sheet according to any one of claims 4 to 6, wherein
the resin particle is a resin particle made of an acrylic resin.

8. The painted steel sheet according to any one of claims 4 to 6, wherein
the binder resin is a binder resin made of an acrylic resin or a polyester resin.

9. The painted steel sheet according to claim 7, wherein
the binder resin is a binder resin made of an acrylic resin or a polyester resin.

10. The painted steel sheet according to claim 1 or 2, having a characteristic selected from any one or two of a surface roughness of the steel sheet being 2 µm or more in Ra on the face of the steel sheet where the 60-degree specular glossiness Gs (60°) is 20% or less, and the paint film layer containing 15% or more of an aggregate composed of a pigment containing silica.
